



US006458524B1

(12) **United States Patent**  
Nakamura et al.

(10) **Patent No.:** US 6,458,524 B1  
(45) **Date of Patent:** Oct. 1, 2002

(54) **SILVER HALIDE PHOTOGRAPHIC LIGHT-SENSITIVE MATERIAL**

(75) Inventors: **Tetsuo Nakamura; Kimiyasu Morimura**, both of Kanagawa (JP)

(73) Assignee: **Fuji Photo Film Co., Ltd.**, Kanagawa (JP)

(\*) Notice: Subject to any disclaimer, the term of this patent is extended or adjusted under 35 U.S.C. 154(b) by 0 days.

(21) Appl. No.: **09/643,717**

(22) Filed: **Aug. 23, 2000**

(30) **Foreign Application Priority Data**

Aug. 31, 1999 (JP) ..... 11-246122

(51) **Int. Cl.<sup>7</sup>** ..... G03C 1/005; G03C 1/494

(52) **U.S. Cl.** ..... 430/584; 430/583; 430/582; 430/581; 430/570

(58) **Field of Search** ..... 430/584, 583, 430/582, 581, 570

(56) **References Cited**

U.S. PATENT DOCUMENTS

- 5,290,676 A 3/1994 Nagaoka et al.  
5,437,972 A \* 8/1995 Ikegawa et al. ..... 430/574  
5,464,734 A \* 11/1995 Inagaki et al. ..... 430/585  
5,464,735 A \* 11/1995 Preddy et al. ..... 430/585  
5,604,089 A \* 2/1997 Ikegawa et al. ..... 430/584  
6,010,842 A \* 1/2000 Suga et al. ..... 430/588

FOREIGN PATENT DOCUMENTS

JP 2000063689 2/2000

\* cited by examiner

*Primary Examiner*—Geraldine Letscher

(74) *Attorney, Agent, or Firm*—Birch, Stewart, Kolasch & Birch, LLP

(57) **ABSTRACT**

A silver halide photographic light-sensitive material is described, comprising at least one compound represented by the following formula (I):



wherein Z<sub>1</sub> and Z<sub>2</sub> each represents oxygen atom, sulfur atom, selenium atom, tellurium atom or a >NR group, R represents an alkyl group, an aryl group or a heterocyclic group, L<sub>1</sub>, L<sub>2</sub> and L<sub>3</sub> each represents a methine group, n<sub>1</sub> represents 0 1, 2 or 3, V<sub>1</sub>, V<sub>2</sub>, V<sub>3</sub>, V<sub>4</sub>, W<sub>1</sub>, W<sub>2</sub>, W<sub>3</sub> and W<sub>4</sub> each represents hydrogen atom or a substituent, provided that two substituents may be combined with each other to form a condensed ring on the condition that assuming the sum total of  $\pi$  values of the substituents V<sub>1</sub> to V<sub>4</sub> is  $\pi_v$  and the sum total of  $\pi$  values of the substituents W<sub>1</sub> to W<sub>4</sub> is  $\pi_w$ , either one of  $\pi_v$  and  $\pi_w$  is 0.70 or less, M represents a charge-balancing counter ion, m represents a number necessary for neutralizing the electric charge of the molecule, R<sub>1</sub> represents an alkyl group, an aryl group or a heterocyclic group, and R<sub>2</sub> represents a substituent represented by any of the following formulae:



wherein R<sub>a</sub>, R<sub>b</sub>, R<sub>c</sub> and R<sub>d</sub> each represents an alkyl group, an aryl group, a heterocyclic group, an alkoxy group, an aryloxy group, a heterocyclyloxy group or an amino group, L<sub>a</sub>, L<sub>b</sub>, L<sub>c</sub>, L<sub>d</sub> and L<sub>e</sub> each represents a methylene group, and k<sub>a</sub>, k<sub>b</sub>, k<sub>c</sub>, k<sub>d</sub> and k<sub>e</sub> each represents an integer of 1 or more.

**7 Claims, No Drawings**

## SILVER HALIDE PHOTOGRAPHIC LIGHT-SENSITIVE MATERIAL

### FIELD OF THE INVENTION

The present invention relates to a silver halide photographic light-sensitive material containing a novel compound, more specifically, the present invention relates to a silver halide photographic light-sensitive material having high sensitivity and reduced in the residual color.

### BACKGROUND OF THE INVENTION

Heretofore, a great deal of efforts have been made to increase the sensitivity of silver halide photographic light-sensitive materials and reduce the persistent coloring (residual color or dye stain). Sensitizing dyes used for the spectral sensitization are known to have great effect on the capabilities of a silver halide photographic light-sensitive material. A slight difference in the structure of sensitizing dyes greatly affects the photographic capabilities such as sensitivity, fog, storage stability and residual color, however, this effect cannot be easily anticipated in advance. Therefore, many researchers have conventionally labored to synthesize a large number of sensitizing dyes and examine the photographic capabilities thereof.

The silver halide tabular grain (hereinafter referred to as a "tabular grain") has the following photographic properties:

- 1) the ratio of the surface area to the volume is large and a large amount of a sensitizing dye can be adsorbed to the surface, so that higher spectral sensitization sensitivity can be obtained;
- 2) when an emulsion containing tabular grains is coated and dried, the grains orient in parallel to the support surface, so that the coated layer can be reduced in the thickness and good sharpness can be obtained;
- 3) the tabular grains oriented in parallel to the support maintain their shape and orientation after the development, so that the developed silver can exhibit high covering power; by virtue of this property, particularly in the case of an X-ray film, the coated silver amount necessary for obtaining an optical density of the same level as otherwise can be reduced;
- 4) the tabular grains oriented in parallel to the support reduce the light scattering, so that an image having high resolution can be obtained; and
- 5) the sensitivity to blue light is low, so that when the silver halide tabular grain is used in a green- or red-sensitive layer, a yellow filter can be reduced or dispensed with.

U.S. Pat. No. 4,439,520 describes a color photographic light-sensitive material improved in the sharpness, sensitivity and graininess by using a tabular grain having a thickness of less than 0.3  $\mu\text{m}$ , a diameter of 0.6  $\mu\text{m}$  or more and an aspect ratio of 8 or more in at least one of the green-sensitive emulsion layer and the red-sensitive emulsion layer. The aspect ratio as used herein means a ratio of the diameter of a tabular grain to the thickness. The diameter of a tabular grain as used herein means a diameter of a circle having the same area as the projected area of a grain when the emulsion is observed through a microscope or an electron microscope. The thickness as used herein is a distance between two parallel planes constituting a tabular grain.

U.S. Pat. No. 4,693,964 describes a photographic element containing silver bromide or silver iodobromide tabular grains having an average diameter of from 0.4 to 0.55  $\mu\text{m}$  and an aspect ratio of 8 or more, where a tabular grain

having an average diameter of 0.5  $\mu\text{m}$  and a thickness of 0.04  $\mu\text{m}$  is disclosed in the Examples. U.S. Pat. No. 4,672,027 describes a photographic element containing silver bromide or silver iodobromide tabular grains having an average diameter of from 0.22 to 0.55  $\mu\text{m}$  and an aspect ratio of 8 or more, where a tabular grain having a thickness of 0.04  $\mu\text{m}$  is disclosed in the Examples.

U.S. Pat. No. 5,250,403 describes a color photographic element containing tabular grains having a (111) main plane, an average diameter of 0.7  $\mu\text{m}$  or more and an average thickness of less than 0.07  $\mu\text{m}$  in a minus blue (green and/or red) layer. Tabular grains having an average thickness of less than 0.07  $\mu\text{m}$  are called an "ultra-thin" tabular grain. In this patent publication, it is stated that the ultra-thin tabular grain emulsion is advantageous in view of the relationship between the sensitivity and the graininess and that this emulsion is preferably used in a color photographic element, particularly, in a minus blue recording emulsion layer, because an image having good sharpness can be obtained.

European Patent 362699 describes a tabular grain in which the ratio of the aspect ratio to the diameter of a tabular grain is larger than 0.7, where a tabular grain having a thickness of 0.04  $\mu\text{m}$  is prepared in the Examples.

As such, investigations have been heretofore concentrated on the development of tabular grains having a higher aspect ratio and a smaller thickness so as to bring out the characteristic properties of the tabular grain to a higher extent. However, requirements for higher quality photographs are strong and development of techniques for achieving still higher sensitivity is keenly demanded.

As described above, the tabular grain is large in the ratio of the surface area to the volume, therefore, a large amount of a sensitizing dye can be adsorbed to the surface and thereby a higher spectral sensitization sensitivity can be obtained. Here, it is considered that by increasing the photoabsorption factor of a sensitizing dye, the efficiency in the transmission of light energy to silver halide can be increased and in turn higher spectral sensitivity can be attained.

In this way, the tabular grain is advantageous for obtaining a high spectral sensitization sensitivity but has a problem in that due to adsorption of a sensitizing dye in a large amount, the residual color after the processing increases. Thus, it is demanded to solve this problem.

From these reasons, studies are being made for a sensitizing dye having high sensitivity and reduced in the residual color.

### SUMMARY OF THE INVENTION

The object of the present invention is to provide a silver halide light-sensitive material having high sensitivity and excellent storage stability and reduced in the fogging and the residual color.

As a result of extensive investigations, the object of the present invention can be attained by the following means:

- (1) a silver halide photographic light-sensitive material comprising a support having provided thereon at least one emulsion layer containing silver halide grains, which comprises at least one compound represented by the following formula (I):



wherein  $Z_1$  and  $Z_2$  each represents oxygen atom, sulfur atom, selenium atom, tellurium atom or a  $>NR$  group (wherein R represents an alkyl group, an aryl group or a heterocyclic group),  $L_1$ ,  $L_2$  and  $L_3$  each represents a methine group,  $n_1$  represents 0, 1, 2 or 3,  $V_1$ ,  $V_2$ ,  $V_3$ ,  $V_4$ ,  $W_1$ ,  $W_2$ ,  $W_3$  and  $W_4$  each represents hydrogen atom or a substituent, provided that two substituents may be combined with each other to form a condensed ring on the condition that assuming the sum total of  $\pi$  values of the substituents  $V_1$  to  $V_4$  is  $\pi_v$  and the sum total of  $\pi$  values of the substituents  $W_1$  to  $W_4$  is  $\pi_w$ , either one of  $\pi_v$  and  $\pi_w$  is 0.70 or less, M represents a charge-balancing counter ion, m represents a number necessary for neutralizing the electric charge of the molecule,  $R_1$  represents an alkyl group, an aryl group or a heterocyclic group, and  $R_2$  represents a substituent represented by any of the following formulae:



wherein  $R_a$ ,  $R_b$ ,  $R_c$  and  $R_d$  each represents an alkyl group, an aryl group, a heterocyclic group, an alkoxy group, an aryloxy group, a heterocyclyloxy group or an amino group,  $L_a$ ,  $L_b$ ,  $L_c$ ,  $L_d$  and  $L_e$  each represents a methylene group, and  $k_a$ ,  $k_b$ ,  $k_c$ ,  $k_d$  and  $k_e$  each represents an integer of 1 or more;

- (2) the silver halide photographic light-sensitive material as described in (1), wherein the sum of  $\pi_v$  and  $\pi_w$  is 1.40 or less;
- (3) the silver halide photographic light-sensitive material as described in (1) or (2), wherein either one of  $\pi_v$  and  $\pi_w$  is 0.70 or more and the other is 0.70 or less;
- (4) the silver halide photographic light-sensitive material as described in (3), wherein  $\pi_v$  is 0.70 or less and  $\pi_w$  is 0.70 or more;
- (5) the silver halide photographic light-sensitive material as described in (4), wherein  $\pi_v$  is from 0.00 to 0.70 and  $\pi_w$  is 0.70 to 1.40;
- (6) the silver halide photographic light-sensitive material as described in (1), wherein the substituent  $R_2$  in the compound represented by formula (I) is  $-(L_e)_{ke}COOH$ ;
- (7) the silver halide photographic light-sensitive material as described in (6), wherein the compound represented by formula (I) is a compound represented by the following formula (II):



wherein  $Z_3$  and  $Z_4$  each represents oxygen atom or sulfur atom,  $A_1$  represents hydrogen atom or an alkyl group, either one of  $V_5$  and  $W_5$  is a substituent selected from the group consisting of chlorine atom, bromine atom, iodine atom, a trifluoromethyl group, an ethyl group, a benzoyl group and a 1-pyrrolyl group, and the other is a substituent selected from the group consisting of hydrogen atom, fluorine atom, a methyl group, a methylthio group, an ethoxy group, an ethoxycarbonyl group, a 2-pyridyl group and a 4-pyridyl group,  $M_1$  represents a charge-balancing counter ion,  $m_1$  represents a number necessary for neutralizing the electric charge of the molecule,  $R_3$  represents an alkyl group having a sulfo group as a substituent,  $L_f$  represents a methylene group, and  $k_f$  represents an integer of from 1 to 3;

- (8) the silver halide photographic light-sensitive material as described in (1), wherein the substituent  $R_2$  in the compound represented by formula (I) is a substituent selected from the group consisting of  $-(L_a)_{ka}CONHSO_2R_a$ ,  $-(L_b)_{kb}SO_2NHCOR_b$ ,  $-(L_c)_{kc}CONHCOR_c$  and  $-(L_d)_{kd}SO_2NHSO_2R_d$ ;
- (9) the silver halide photographic light-sensitive material as described in (8), wherein the compound represented by formula (I) is a compound represented by the following formula (III):



wherein  $Z_5$  and  $Z_6$  each represents oxygen atom or sulfur atom,  $A_2$  represents hydrogen atom or an alkyl group,  $V_6$  represents a substituent selected from the group consisting of hydrogen atom, fluorine atom, a methyl group, a methylthio group, an ethoxy group, an ethoxycarbonyl group, a 2-pyridyl group and a 4-pyridyl group,  $W_6$  represents a substituent selected from the group consisting of chlorine atom, bromine atom, iodine atom, a trifluoromethyl group, an ethyl group, a benzoyl group and a 1-pyrrolyl group,  $M_2$  represents a charge-balancing counter ion,  $m_2$  represents a number necessary for neutralizing the electric charge of the molecule,  $R_4$  represents an alkyl group having a sulfo group as a substituent,  $R_g$  represents an alkyl group,  $L_g$  represents a methylene group, and  $k_g$  represents an integer of from 1 to 3; and

- (10) the silver halide photographic light-sensitive material as described in (1), (2), (3), (4), (5), (6), (7), (8) or (9),

wherein at least one compound represented by formula (I), (II) or (III) is contained and the emulsion layer containing the compound is formed of silver halide grains having an average aspect ratio of from 3 to 100.

#### DETAILED DESCRIPTION OF THE INVENTION

The compound represented by formula (I) for use in the present invention is described in detail below.

$Z_1$  and  $Z_2$  each represents oxygen atom, sulfur atom, selenium atom, tellurium atom or a  $>NR$  group, R represents an alkyl group, an aryl group or a heterocyclic group, and  $R_1$  represents an alkyl group, an aryl group or a heterocyclic group.

Examples of the alkyl group represented by R or  $R_1$  include an unsubstituted alkyl group having from 1 to 8, preferably from 1 to 4, carbon atoms (e.g., methyl, ethyl, propyl, isopropyl, butyl, isobutyl, hexyl), and an alkyl group having from 1 to 8, preferably from 1 to 4, carbon atoms, which is substituted by V described below {examples of V include a halogen atom (e.g., chlorine, bromine, iodine, fluorine), a mercapto group, a cyano group, a carboxyl group, a phosphoric acid group, a sulfo group, a hydroxy group, a carbamoyl group having from 1 to 7, preferably from 2 to 5, more preferably from 2 to 3, carbon atoms (e.g., methylcarbamoyl, ethylcarbamoyl, morpholinocarbonyl), a sulfamoyl group having from 0 to 7, preferably from 2 to 5, more preferably from 2 to 3 carbon atoms (e.g., methylsulfamoyl, ethylsulfamoyl, piperidinosulfonyl), a nitro group, an alkoxy group having from 1 to 7, preferably from 1 to 5, more preferably from 1 to 3, carbon atoms (e.g., methoxy, ethoxy, 2-methoxyethoxy, 2-phenylethoxy), an aryloxy group having from 6 to 7 carbon atoms (e.g., phenoxy, p-methylphenoxy, p-chlorophenoxy), an acyl group having from 1 to 7, preferably from 2 to 5, more preferably from 2 to 3, carbon atoms (e.g., acetyl, benzoyl, trichloroacetyl), an acyloxy group having from 1 to 7, preferably from 2 to 5, more preferably from 2 to 3, carbon atoms (e.g., acetoxy, benzyloxy), an acylamino group having from 1 to 7, preferably from 2 to 5, more preferably from 2 to 3, carbon atoms (e.g., acetylamino), a sulfonyl group having from 1 to 7, preferably from 1 to 5, more preferably from 1 to 3, carbon atoms (e.g., methanesulfonyl, ethanesulfonyl, benzenesulfonyl), a sulfinyl group having from 1 to 7, preferably from 1 to 5, more preferably from 1 to 3, carbon atoms (e.g., methanesulfinyl, benzenesulfinyl), a sulfonamino group having from 1 to 7, preferably from 1 to 5, more preferably from 1 to 3, carbon atoms (e.g., methanesulfonylamino, ethanesulfonylamino, benzenesulfonylamino), an amino group, a substituted amino group having from 1 to 7, preferably from 1 to 5, more preferably from 1 to 3, carbon atoms (e.g., methylamino, dimethylamino, benzylamino, anilino), an ammonium group having from 0 to 7, preferably from 0 to 5, more preferably from 0 to 3, carbon atoms (e.g., trimethylammonium, triethylammonium), a hydrazino group having from 0 to 7, preferably from 1 to 5, more preferably from 1 to 3, carbon atoms (e.g., trimethylhydrazino), a ureido group having from 1 to 7, preferably from 1 to 5, more preferably from 1 to 3, carbon atoms (e.g., ureido, N,N-dimethylureido), an imido group having from 1 to 7, preferably from 1 to 5, more preferably from 1 to 3, carbon atoms (e.g., succinimido), an alkyl- or aryl-thio group having from 1 to 7, preferably from 1 to 5, more preferably from 1 to 3, carbon atoms (e.g., methylthio, ethylthio, carboxyethylthio, sulfobutylthio, phenylthio), an alkoxycarbonyl group having from 2 to 7, preferably from 2

to 5, more preferably from 2 to 3, carbon atoms (e.g., methoxycarbonyl, ethoxycarbonyl, benzyloxycarbonyl), an aryloxycarbonyl group having from 6 to 7 carbon atoms (e.g., phenoxy carbonyl), an unsubstituted alkyl group having from 1 to 7, preferably from 1 to 5, more preferably from 1 to 3, carbon atoms (e.g., methyl, ethyl, propyl, butyl), a substituted alkyl group having from 1 to 7, preferably from 1 to 5, more preferably from 1 to 3, carbon atoms (e.g., hydroxymethyl, trifluoromethyl, benzyl, carboxyethyl, ethoxycarbonylmethyl, acetylamino-methyl; the substituted alkyl group as used herein also includes an unsaturated hydrocarbon group preferably having from 2 to 7, more preferably from 2 to 5, still more preferably from 2 to 3, carbon atoms (e.g., vinyl, ethynyl, 1-cyclohexenyl, benzylidene, benzylidene)), a substituted or unsubstituted aryl group having from 6 to 7 carbon atoms (e.g., phenyl, p-carboxyphenyl, p-nitrophenyl, 3,5-dichlorophenyl, p-cyanophenyl, m-fluorophenyl, p-tolyl) and a heterocyclic group having from 1 to 7, preferably from 2 to 5, carbon atoms (e.g., pyridyl, 5-methylpyridyl, thiienyl, furyl, morpholino, tetrahydrofurfuryl); two of these substituents may be combined with each other to have a structure where a benzene ring, a naphthalene ring, an anthracene ring or a heterocyclic ring is condensed; these substituents each may be further substituted by V thereon}.

Examples of the aryl group represented by R or  $R_1$  include an unsubstituted aryl group having from 6 to 20, preferably from 6 to 10, more preferably from 6 to 8, carbon atoms (e.g., phenyl, 1-naphthyl), and a substituted aryl group having from 6 to 20, preferably from 6 to 10, more preferably from 6 to 8, carbon atoms (e.g., the above-described aryl group substituted by V, specifically, p-methoxyphenyl group, p-methylphenyl, p-chlorophenyl).

Examples of the heterocyclic group represented by R or  $R_1$  include an unsubstituted heterocyclic group having from 1 to 20, preferably from 3 to 10, more preferably from 4 to 8, carbon atoms (e.g., 2-furyl, 2-thienyl, 2-pyridyl, 3-pyrazolyl, 3-isooxazolyl, 3-isothiazolyl, 2-imidazolyl, 2-oxazolyl, 2-thiazolyl, 2-pyridazyl, 2-pyrimidyl, 3-pyrazyl, 2-(1,3,5-triazolyl), 3-(1,2,4-triazolyl), 5-tetrazolyl), and a substituted heterocyclic group having from 1 to 20, preferably from 3 to 10, more preferably from 4 to 8, carbon atoms (e.g., the above-described heterocyclic group substituted by V, specifically, 5-methyl-2-thienyl, 4-methoxy-2-pyridyl).

R is preferably an alkyl group, more preferably a substituted or unsubstituted alkyl group having from 1 to 6 carbon atoms, still more preferably an unsubstituted alkyl group having from 1 to 4 carbon atoms.

$Z_1$  and  $Z_2$  each is preferably oxygen atom or sulfur atom, and at least one of  $Z_1$  and  $Z_2$  is more preferably sulfur atom.

$R_1$  is preferably an alkyl group, more preferably an alkyl group having an acidic group (for example, a sulfo group, a carboxyl group, a sulfato group, a phosphono group, a borono group or a substituent described above for  $R_2$ ), still more preferably an alkyl group having from 1 to 6 carbon atoms and having a sulfo group, particularly preferably a sulfoalkyl group having from 2 to 4 carbon atoms.

The methine group represented by  $L_1$ ,  $L_2$  or  $L_3$  may be unsubstituted or substituted and when substituted, examples of the substituent are the same as those of the substituent V.

$n_1$  is 0, 1 or 2 and when  $n_1$  is 2, two pairs of  $L_2$  and  $L_3$  may be the same or different. Also, two methine groups may be combined with each other to form a ring.

In a preferred embodiment of the compound,  $n_1$  is 1,  $L_1$  and  $L_3$  each is an unsubstituted methine group, and  $L_2$  is a methine group substituted by an alkyl group. The alkyl

group on the methine group represented by  $L_2$  is preferably a substituted or unsubstituted alkyl group having from 1 to 4 carbon atoms, more preferably methyl or ethyl.

$V_1$ ,  $V_2$ ,  $V_3$ ,  $V_4$ ,  $W_1$ ,  $W_2$ ,  $W_3$  and  $W_4$  each represents hydrogen atom or a substituent and two of these substituents may be combined with each other to form a condensed ring.

The  $\pi$  value used in the present invention is described below. The  $\pi$  value is a parameter showing the effect of a substituent upon the hydrophilicity/hydrophobicity of a molecule of a compound and is defined by the following formula:

$$\pi = \log P(\text{PhX}) - \log P(\text{PhH})$$

wherein P is a distribution coefficient of the compound to octanol/water and the difference between the logP value of substituted benzene  $\text{PhX}$  and the logP value of benzene is assigned to the  $\pi$  value of the substituent X. The logP value can be determined based on the actual measurement according to the method described in the following publication (a) or can be determined by the calculation using the fragment method described in the publication (a) or the software package described in the publication (b). In the case where the found value does not agree with the calculated value, the found  $\pi$  value is used in principle.

(a) C. Hansch and A. J. Leo, *Substituent Constants for Correlation Analysis in Chemistry and Biology*, John Wiley & Sons, New York (1979)

(b) Medicem software package (Ver. 3.54) developed by and available from Pomona College, Claremont, Calif.

Incidentally, for example, when  $V_1$  and  $V_2$  are combined with each other to form a naphthalene ring system, the  $\pi$  value assigned to  $V_1$  and  $V_2$  can be determined as follows by regarding the  $-\text{CH}=\text{CH}-\text{CH}=\text{CH}-$  as a substituent. The same applies to other condensed rings.

$$\pi(-(\text{CH})_4-) = \log P(\text{naphthalene}) - \log P(\text{benzene}) = 1.32$$

The  $\pi$  values of respective substituents determined as above are listed in the publication (a). Main substituents are selected and their  $\pi$  values are shown below.

| Substituent                   | $\pi$ value |
|-------------------------------|-------------|
| OH                            | -0.67       |
| CN                            | -0.57       |
| COCH <sub>3</sub>             | -0.55       |
| COOH                          | -0.32       |
| OCH <sub>3</sub>              | -0.02       |
| COOCH <sub>3</sub>            | -0.01       |
| H                             | 0.00        |
| F                             | 0.14        |
| CH <sub>3</sub>               | 0.56        |
| Cl                            | 0.71        |
| Br                            | 0.86        |
| I                             | 1.12        |
| -(CH) <sub>4</sub> -          | 1.32        |
| C <sub>6</sub> H <sub>5</sub> | 1.96        |

In the present invention, assuming that the total sum of the  $\pi$  values of the substituents  $V_1$  to  $V_4$  is  $\pi_v$ , and the total sum of the  $\pi$  values of the substituents  $W_1$  to  $W_4$  is  $\pi_w$ , either one of  $\pi_v$  and  $\pi_w$  must be 0.70 or less. The sum of  $\pi_v$  and  $\pi_w$  is preferably 1.40 or less. Furthermore, it is preferred that either one of  $\pi_v$  and  $\pi_w$  is 0.70 or more and the other is 0.70 or less, more preferably one is from 0.70 to 1.40 and the other is from 0.00 to 0.70, still more preferably  $\pi_v$  is 0.70 or less and  $\pi_w$  is 0.70 or more, and most preferably  $\pi_v$  is from 0.00 to 0.70 and  $\pi_w$  is from 0.70 to 1.40.

$R_a$ ,  $R_b$ ,  $R_c$  and  $R_d$  in the group represented by  $R_2$  each represents an alkyl group, an aryl group, a heterocyclic group, an alkoxy group, an aryloxy group, a heterocyclyloxy group or an amino group. Preferred examples thereof are described below.

Preferred examples thereof include an unsubstituted alkyl group having from 1 to 18, preferably from 1 to 10, more preferably from 1 to 5, carbon atoms (e.g., methyl, ethyl, propyl, butyl), a substituted alkyl group having from 1 to 18, preferably from 1 to 10, more preferably from 1 to 5, carbon atoms (e.g., hydroxymethyl, trifluoromethyl, benzyl, carboxyethyl, ethoxycarbonylmethyl, acetylaminomethyl); the substituted alkyl group as used herein also includes an unsaturated hydrocarbon group preferably having from 2 to 18, more preferably from 3 to 10, still more preferably from 3 to 5, carbon atoms (e.g., vinyl, ethynyl, 1-cyclohexenyl, benzylidene, benzylidene), a substituted or unsubstituted aryl group having from 6 to 20, preferably from 6 to 15, more preferably from 6 to 10, carbon atoms (e.g., phenyl, 1-naphthyl, p-carboxyphenyl, p-nitrophenyl, 3,5-dichlorophenyl, p-cyanophenyl, m-fluorophenyl, p-tolyl), a heterocyclic group having from 1 to 20, preferably from 2 to 10, more preferably from 4 to 6, carbon atoms (e.g., pyridyl, 5-methylpyridyl, thiienyl, furyl, morpholino, tetrahydrofuryl), an alkoxy group having from 1 to 10, preferably from 1 to 8, carbon atoms (e.g., methoxy, ethoxy, 2-methoxyethoxy, 2-hydroxyethoxy, 2-phenylethoxy), an aryloxy group having from 6 to 20, preferably from 6 to 12, more preferably from 6 to 10, carbon atoms (e.g., phenoxy, p-methylphenoxy, p-chlorophenoxy, naphthoxy), a heterocyclyloxy group having from 1 to 20, preferably from 3 to 12, more preferably from 3 to 10, carbon atoms (e.g., 2-thienyloxy, 2-morpholinoxy), and an amino group having from 0 to 20, preferably from 0 to 12, more preferably from 0 to 8, carbon group (e.g., amino, methylamino, dimethylamino, ethylamino, diethylamino, hydroxyethylamino, benzylamino, anilino, diphenylamino, morpholino formed into a ring, pyrrolidino). These groups each may be substituted by the substituent V.

Among these, more preferred are methyl, ethyl and hydroxyethyl, still more preferred is methyl.

The methylene group represented by  $L_a$ ,  $L_b$ ,  $L_c$ ,  $L_d$  or  $L_e$  may be unsubstituted or substituted by a substituent and the substituent is not particularly limited but preferred examples thereof include the substituent V.

Specific examples of the substituted methylene group include a methyl-substituted methylene group, an ethyl-substituted methylene group, a phenyl-substituted methylene group, a hydroxy-substituted methylene group and a halogen (e.g., chlorine, bromine)-substituted methylene group. The methylene group is preferably an unsubstituted methylene group.

$k_a$ ,  $k_b$ ,  $k_c$ ,  $k_d$  and  $k_e$  each represents an integer of 1 or more, preferably from 1 to 4, more preferably 1 or 2, still more preferably 1. When  $k_a$ ,  $k_b$ ,  $k_c$ ,  $k_d$  and  $k_e$  each is 2 or more, the repeated  $L_a$ ,  $L_b$ ,  $L_c$ ,  $L_d$  or  $L_e$  may not be the same.

The dissociative groups NH and OH of  $R_2$  are denoted by the non-dissociative form in all cases but these can take a dissociated form ( $\text{N}^-$  or  $\text{O}^-$ ). Actually, these groups assume the dissociated state or the non-dissociated state depending on the environment where the dye is present, such as pH.

With respect to the notation, the group in the dissociated state is denoted, for example, as  $\text{N}^-$ . In the case where a cationic compound (for example, sodium ion) is present as a counter salt, the notation is  $\text{N}^-\text{Na}^+$ . Even in the non-dissociated state, if the cationic compound as a counter salt is regarded as a proton, the notation of  $\text{N}^-\text{H}^+$  may be used.

Preferred examples of  $R_2$  are shown below. In all cases, the dissociative group is denoted by the non-dissociated form.



In the above, the groups positioned earlier are more preferred. Among these, particularly preferred are  $R_{2a}$  and  $R_{2b}$ .

$M$  is contained in the formula so as to show the presence of cation or anion when such ion is necessary for neutralizing the ion charge. Whether a dye is cation or anion or whether or not a dye has a net ion, depends on the substituent. Typical examples of the cation include inorganic cation such as hydrogen ion, alkali metal ion (e.g., sodium ion, potassium ion, lithium ion), alkaline earth metal ion (e.g., calcium ion) and an organic anion such as ammonium ion (e.g., ammonium ion, tetraalkylammonium ion, pyridinium ion, ethylpyridinium ion). The anion may be either inorganic anion or organic anion and examples thereof include halide anion (e.g., fluoride anion, chloride anion, bromide ion, iodide ion), substituted arylsulfonate ion (e.g., p-toluenesulfonate ion, p-chlorobenzenesulfonate ion), aryldisulfonate ion (e.g., 1,3-benzenedisulfonate ion, 2,6-naphthalenedisulfonate ion), alkylsulfate ion (e.g., methylsulfate ion), sulfate ion, thiocyanate ion, perchlorate ion, tetrafluoroborate ion, picrate ion, acetate ion and trifluoromethanesulfonate ion.

Among those cations, preferred are sodium ion, potassium ion, triethylammonium ion, tetraethylammonium ion, pyridinium, ethylpyridinium ion and methylpyridinium ion. Among those anions, preferred are perchlorate ion, iodide ion, bromide ion and substituted arylsulfonate ion (e.g., p-toluenesulfonate ion).

$m$  represents a number of 0 or more necessary for balancing the electric charge in the molecule and when an inner salt is formed,  $m$  is 0.  $m$  is preferably a number of from 0 to 4.

The compound represented by formula (I) is more preferably a compound represented by formula (II) or (III).

The compound represented by formula (II) is described in detail below.

$Z_3$  and  $Z_4$  each represents oxygen atom or sulfur atom. Preferably, at least one of  $Z_3$  and  $Z_4$  is sulfur atom and more preferably, both are sulfur atom.

$A_1$  represents hydrogen atom or an alkyl group and preferred examples of the alkyl group include the unsubstituted or substituted alkyl groups described above for  $R$ . The alkyl group is more preferably a substituted or unsubstituted alkyl group having from 1 to 4 carbon atoms, still more preferably methyl or ethyl.

Either one of  $V_5$  and  $W_5$  is a substituent selected from the group consisting of hydrogen atom, fluorine atom, a methyl group, a methylthio group, an ethoxy group, an ethoxycarbonyl group, a 2-pyridyl group and a 4-pyridyl group, preferably hydrogen atom or fluorine atom. The other is a substituent selected from the group consisting of chlorine atom, bromine atom, iodine atom, a trifluoromethyl group, an ethyl group, a benzoyl group and a 1-pyrrolyl group, preferably chlorine atom or bromine atom.

10 The alkyl group having a sulfo group as a substituent, represented by  $R_3$ , may have a substituent other than the sulfo group. For example, oxygen or other non-carbon atomic group may be interposed between the sulfo group and the alkyl group as in a sulfopropoxyethyl group. The 15 alkyl group is preferably an alkyl group directly substituted by a sulfo group, more preferably a 3-sulfopropyl group, a 3-sulfonyl group or a 4-sulfonyl group.

Preferred examples of the methylene group represented by  $L_f$  are the same as those described above for  $L_a$ . The 20 methylene group is more preferably an unsubstituted methylene group.

$k_f$  is an integer of from 1 to 3, preferably 1 or 2, more preferably 1.

The compound represented by formula (III) is described 25 in detail below.

$Z_5$  and  $Z_6$  each represents oxygen atom or sulfur atom. Preferably, at least one  $Z_5$  and  $Z_6$  is sulfur atom, and more preferably, both are sulfur atom.

$A_2$  represents hydrogen atom or an alkyl group and 30 preferred examples of the alkyl group include those described above as preferred examples of the unsubstituted or substituted alkyl group represented by  $R$ . The alkyl group is more preferably a substituted or unsubstituted alkyl group having from 1 to 4 carbon atoms, still more preferably 35 methyl or ethyl.

$V_6$  is a substituent selected from the group consisting of hydrogen atom, fluorine atom, a mercapto group, a methyl group, a methylthio group, an ethoxy group, an ethoxycarbonyl group, a 2-pyridyl group and a 4-pyridyl group, 40 preferably hydrogen atom or fluorine atom, more preferably fluorine atom.

$W_6$  is a substituent selected from the group consisting of chlorine atom, bromine atom, iodine atom, a trifluoromethyl group, an ethyl group, a benzoyl group and a 1-pyrrolyl group, 45 preferably chlorine atom or bromine atom, more preferably chlorine atom.

$R_4$  represents an alkyl group having a sulfo group as a substituent and preferred examples thereof are the same as those described above for  $R_3$ . The alkyl group is more 50 preferably an alkyl group directly substituted by a sulfo group, still more preferably a 3-sulfopropyl group, a 3-sulfonyl group or a 4-sulfonyl group.

Preferred examples of the alkyl group represented by  $R_g$  55 are the same as those described above for  $R_a$  and the alkyl group is more preferably methyl or ethyl, still more preferably methyl.

Preferred examples of the methylene group represented by  $L_g$  are the same as those described above for  $L_a$  and the 60 methylene group is more preferably an unsubstituted methylene group.

$k_g$  is an integer of from 1 to 3, preferably 1 or 2, more preferably 1.

Specific examples of the compounds represented by formulas (I), (II) and (III) of the present invention are shown 65 below, however, the present invention is by no means limited thereto.

11



12



-continued  
I-15



I-17



I-19



K<sup>+</sup>

I-21



I-22



I-23



I-24

I-25



continued  
I-26

II-1



The compounds represented by formulae (I), (II) and (III) of the present invention can be synthesized according to the methods described in the following publications:

- a) F. M. Harmer, *Heterocyclic Compounds-Cyanine dyes and related compounds*, John Wiley & Sons, New York, London (1964);  
 b) D. M. Sturmer, *Heterocyclic Compounds-Special topics in heterocyclic chemistry*, Chap. 8, Sec. 4, pp. 482-515, John Wiley & Sons, New York, London (1977); and

c) *Rodd's Chemistry of Carbon Compounds*, 2nd ver. Vol. 4, part B, Chap. 15, pp. 369-422, Elsevier Science Publishing Company Inc., New York (1977).

60  
 65  
 66  
 67  
 68  
 69  
 70  
 71  
 72  
 73  
 74  
 75  
 76  
 77  
 78  
 79  
 80  
 81  
 82  
 83  
 84  
 85  
 86  
 87  
 88  
 89  
 90  
 91  
 92  
 93  
 94  
 95  
 96  
 97  
 98  
 99  
 100  
 101  
 102  
 103  
 104  
 105  
 106  
 107  
 108  
 109  
 110  
 111  
 112  
 113  
 114  
 115  
 116  
 117  
 118  
 119  
 120  
 121  
 122  
 123  
 124  
 125  
 126  
 127  
 128  
 129  
 130  
 131  
 132  
 133  
 134  
 135  
 136  
 137  
 138  
 139  
 140  
 141  
 142  
 143  
 144  
 145  
 146  
 147  
 148  
 149  
 150  
 151  
 152  
 153  
 154  
 155  
 156  
 157  
 158  
 159  
 160  
 161  
 162  
 163  
 164  
 165  
 166  
 167  
 168  
 169  
 170  
 171  
 172  
 173  
 174  
 175  
 176  
 177  
 178  
 179  
 180  
 181  
 182  
 183  
 184  
 185  
 186  
 187  
 188  
 189  
 190  
 191  
 192  
 193  
 194  
 195  
 196  
 197  
 198  
 199  
 200  
 201  
 202  
 203  
 204  
 205  
 206  
 207  
 208  
 209  
 210  
 211  
 212  
 213  
 214  
 215  
 216  
 217  
 218  
 219  
 220  
 221  
 222  
 223  
 224  
 225  
 226  
 227  
 228  
 229  
 230  
 231  
 232  
 233  
 234  
 235  
 236  
 237  
 238  
 239  
 240  
 241  
 242  
 243  
 244  
 245  
 246  
 247  
 248  
 249  
 250  
 251  
 252  
 253  
 254  
 255  
 256  
 257  
 258  
 259  
 260  
 261  
 262  
 263  
 264  
 265  
 266  
 267  
 268  
 269  
 270  
 271  
 272  
 273  
 274  
 275  
 276  
 277  
 278  
 279  
 280  
 281  
 282  
 283  
 284  
 285  
 286  
 287  
 288  
 289  
 290  
 291  
 292  
 293  
 294  
 295  
 296  
 297  
 298  
 299  
 300  
 301  
 302  
 303  
 304  
 305  
 306  
 307  
 308  
 309  
 310  
 311  
 312  
 313  
 314  
 315  
 316  
 317  
 318  
 319  
 320  
 321  
 322  
 323  
 324  
 325  
 326  
 327  
 328  
 329  
 330  
 331  
 332  
 333  
 334  
 335  
 336  
 337  
 338  
 339  
 340  
 341  
 342  
 343  
 344  
 345  
 346  
 347  
 348  
 349  
 350  
 351  
 352  
 353  
 354  
 355  
 356  
 357  
 358  
 359  
 360  
 361  
 362  
 363  
 364  
 365  
 366  
 367  
 368  
 369  
 370  
 371  
 372  
 373  
 374  
 375  
 376  
 377  
 378  
 379  
 380  
 381  
 382  
 383  
 384  
 385  
 386  
 387  
 388  
 389  
 390  
 391  
 392  
 393  
 394  
 395  
 396  
 397  
 398  
 399  
 400  
 401  
 402  
 403  
 404  
 405  
 406  
 407  
 408  
 409  
 410  
 411  
 412  
 413  
 414  
 415  
 416  
 417  
 418  
 419  
 420  
 421  
 422  
 423  
 424  
 425  
 426  
 427  
 428  
 429  
 430  
 431  
 432  
 433  
 434  
 435  
 436  
 437  
 438  
 439  
 440  
 441  
 442  
 443  
 444  
 445  
 446  
 447  
 448  
 449  
 450  
 451  
 452  
 453  
 454  
 455  
 456  
 457  
 458  
 459  
 460  
 461  
 462  
 463  
 464  
 465  
 466  
 467  
 468  
 469  
 470  
 471  
 472  
 473  
 474  
 475  
 476  
 477  
 478  
 479  
 480  
 481  
 482  
 483  
 484  
 485  
 486  
 487  
 488  
 489  
 490  
 491  
 492  
 493  
 494  
 495  
 496  
 497  
 498  
 499  
 500  
 501  
 502  
 503  
 504  
 505  
 506  
 507  
 508  
 509  
 510  
 511  
 512  
 513  
 514  
 515  
 516  
 517  
 518  
 519  
 520  
 521  
 522  
 523  
 524  
 525  
 526  
 527  
 528  
 529  
 530  
 531  
 532  
 533  
 534  
 535  
 536  
 537  
 538  
 539  
 540  
 541  
 542  
 543  
 544  
 545  
 546  
 547  
 548  
 549  
 550  
 551  
 552  
 553  
 554  
 555  
 556  
 557  
 558  
 559  
 560  
 561  
 562  
 563  
 564  
 565  
 566  
 567  
 568  
 569  
 570  
 571  
 572  
 573  
 574  
 575  
 576  
 577  
 578  
 579  
 580  
 581  
 582  
 583  
 584  
 585  
 586  
 587  
 588  
 589  
 590  
 591  
 592  
 593  
 594  
 595  
 596  
 597  
 598  
 599  
 600  
 601  
 602  
 603  
 604  
 605  
 606  
 607  
 608  
 609  
 610  
 611  
 612  
 613  
 614  
 615  
 616  
 617  
 618  
 619  
 620  
 621  
 622  
 623  
 624  
 625  
 626  
 627  
 628  
 629  
 630  
 631  
 632  
 633  
 634  
 635  
 636  
 637  
 638  
 639  
 640  
 641  
 642  
 643  
 644  
 645  
 646  
 647  
 648  
 649  
 650  
 651  
 652  
 653  
 654  
 655  
 656  
 657  
 658  
 659  
 660  
 661  
 662  
 663  
 664  
 665  
 666  
 667  
 668  
 669  
 670  
 671  
 672  
 673  
 674  
 675  
 676  
 677  
 678  
 679  
 680  
 681  
 682  
 683  
 684  
 685  
 686  
 687  
 688  
 689  
 690  
 691  
 692  
 693  
 694  
 695  
 696  
 697  
 698  
 699  
 700  
 701  
 702  
 703  
 704  
 705  
 706  
 707  
 708  
 709  
 710  
 711  
 712  
 713  
 714  
 715  
 716  
 717  
 718  
 719  
 720  
 721  
 722  
 723  
 724  
 725  
 726  
 727  
 728  
 729  
 730  
 731  
 732  
 733  
 734  
 735  
 736  
 737  
 738  
 739  
 740  
 741  
 742  
 743  
 744  
 745  
 746  
 747  
 748  
 749  
 750  
 751  
 752  
 753  
 754  
 755  
 756  
 757  
 758  
 759  
 760  
 761  
 762  
 763  
 764  
 765  
 766  
 767  
 768  
 769  
 770  
 771  
 772  
 773  
 774  
 775  
 776  
 777  
 778  
 779  
 780  
 781  
 782  
 783  
 784  
 785  
 786  
 787  
 788  
 789  
 790  
 791  
 792  
 793  
 794  
 795  
 796  
 797  
 798  
 799  
 800  
 801  
 802  
 803  
 804  
 805  
 806  
 807  
 808  
 809  
 810  
 811  
 812  
 813  
 814  
 815  
 816  
 817  
 818  
 819  
 820  
 821  
 822  
 823  
 824  
 825  
 826  
 827  
 828  
 829  
 830  
 831  
 832  
 833  
 834  
 835  
 836  
 837  
 838  
 839  
 840  
 841  
 842  
 843  
 844  
 845  
 846  
 847  
 848  
 849  
 850  
 851  
 852  
 853  
 854  
 855  
 856  
 857  
 858  
 859  
 860  
 861  
 862  
 863  
 864  
 865  
 866  
 867  
 868  
 869  
 870  
 871  
 872  
 873  
 874  
 875  
 876  
 877  
 878  
 879  
 880  
 881  
 882  
 883  
 884  
 885  
 886  
 887  
 888  
 889  
 890  
 891  
 892  
 893  
 894  
 895  
 896  
 897  
 898  
 899  
 900  
 901  
 902  
 903  
 904  
 905  
 906  
 907  
 908  
 909  
 910  
 911  
 912  
 913  
 914  
 915  
 916  
 917  
 918  
 919  
 920  
 921  
 922  
 923  
 924  
 925  
 926  
 927  
 928  
 929  
 930  
 931  
 932  
 933  
 934  
 935  
 936  
 937  
 938  
 939  
 940  
 941  
 942  
 943  
 944  
 945  
 946  
 947  
 948  
 949  
 950  
 951  
 952  
 953  
 954  
 955  
 956  
 957  
 958  
 959  
 960  
 961  
 962  
 963  
 964  
 965  
 966  
 967  
 968  
 969  
 970  
 971  
 972  
 973  
 974  
 975  
 976  
 977  
 978  
 979  
 980  
 981  
 982  
 983  
 984  
 985  
 986  
 987  
 988  
 989  
 990  
 991  
 992  
 993  
 994  
 995  
 996  
 997  
 998  
 999  
 1000  
 1001  
 1002  
 1003  
 1004  
 1005  
 1006  
 1007  
 1008  
 1009  
 1010  
 1011  
 1012  
 1013  
 1014  
 1015  
 1016  
 1017  
 1018  
 1019  
 1020  
 1021  
 1022  
 1023  
 1024  
 1025  
 1026  
 1027  
 1028  
 1029  
 1030  
 1031  
 1032  
 1033  
 1034  
 1035  
 1036  
 1037  
 1038  
 1039  
 1040  
 1041  
 1042  
 1043  
 1044  
 1045  
 1046  
 1047  
 1048  
 1049  
 1050  
 1051  
 1052  
 1053  
 1054  
 1055  
 1056  
 1057  
 1058  
 1059  
 1060  
 1061  
 1062  
 1063  
 1064  
 1065  
 1066  
 1067  
 1068  
 1069  
 1070  
 1071  
 1072  
 1073  
 1074  
 1075  
 1076  
 1077  
 1078  
 1079  
 1080  
 1081  
 1082  
 1083  
 1084  
 1085  
 1086  
 1087  
 1088  
 1089  
 1090  
 1091  
 1092  
 1093  
 1094  
 1095  
 1096  
 1097  
 1098  
 1099  
 1100  
 1101  
 1102  
 1103  
 1104  
 1105  
 1106  
 1107  
 1108  
 1109  
 1110  
 1111  
 1112  
 1113  
 1114  
 1115  
 1116  
 1117  
 1118  
 1119  
 1120  
 1121  
 1122  
 1123  
 1124  
 1125  
 1126  
 1127  
 1128  
 1129  
 1130  
 1131  
 1132  
 1133  
 1134  
 1135  
 1136  
 1137  
 1138  
 1139  
 1140  
 1141  
 1142  
 1143  
 1144  
 1145  
 1146  
 1147  
 1148  
 1149  
 1150  
 1151  
 1152  
 1153  
 1154  
 1155  
 1156  
 1157  
 1158  
 1159  
 1160  
 1161  
 1162  
 1163  
 1164  
 1165  
 1166  
 1167  
 1168  
 1169  
 1170  
 1171  
 1172  
 1173  
 1174  
 1175  
 1176  
 1177  
 1178  
 1179  
 1180  
 1181  
 1182  
 1183  
 1184  
 1185  
 1186  
 1187  
 1188  
 1189  
 1190  
 1191  
 1192  
 1193  
 1194  
 1195  
 1196  
 1197  
 1198  
 1199  
 1200  
 1201  
 1202  
 1203  
 1204  
 1205  
 1206  
 1207  
 1208  
 1209  
 1210  
 1211  
 1212  
 1213  
 1214  
 1215  
 1216  
 1217  
 1218  
 1219  
 1220  
 1221  
 1222  
 1223  
 1224  
 1225  
 1226  
 1227  
 1228  
 1229  
 1230  
 1231  
 1232  
 1233  
 1234  
 1235  
 1236  
 1237  
 1238  
 1239  
 1240  
 1241  
 1242  
 1243  
 1244  
 1245  
 1246  
 1247  
 1248  
 1249  
 1250  
 1251  
 1252  
 1253  
 1254  
 1255  
 1256  
 1257  
 1258  
 1259  
 1260  
 1261  
 1262  
 1263  
 1264  
 1265  
 1266  
 1267  
 1268  
 1269  
 1270  
 1271  
 1272  
 1273  
 1274  
 1275  
 1276  
 1277  
 1278  
 1279  
 1280  
 1281  
 1282  
 1283  
 1284  
 1285  
 1286  
 1287  
 1288  
 1289  
 1290  
 1291  
 1292  
 1293  
 1294  
 1295  
 1296  
 1297  
 1298  
 1299  
 1300  
 1301  
 1302  
 1303  
 1304  
 1305  
 1306  
 1307  
 1308  
 1309  
 1310  
 1311  
 1312  
 1313  
 1314  
 1315  
 1316  
 1317  
 1318  
 1319  
 1320  
 1321  
 1322  
 1323  
 1324  
 1325  
 1326  
 1327  
 1328  
 1329  
 1330  
 1331  
 1332  
 1333  
 1334  
 1335  
 1336  
 1337  
 1338  
 1339  
 1340  
 1341  
 1342  
 1343  
 1344  
 1345  
 1346  
 1347  
 1348  
 1349  
 1350  
 1351  
 1352  
 1353  
 1354  
 1355  
 1356  
 1357  
 1358  
 1359  
 1360  
 1361  
 1362  
 1363  
 1364  
 1365  
 1366  
 1367  
 1368  
 1369  
 1370  
 1371  
 1372  
 1373  
 1374  
 1375  
 1376  
 1377  
 1378  
 1379  
 1380  
 1381  
 1382  
 1383  
 1384  
 1385  
 1386  
 1387  
 1388  
 1389  
 1390  
 1391  
 1392  
 1393  
 1394  
 1395  
 1396  
 1397  
 1398  
 1399  
 1400  
 1401  
 1402  
 1403  
 1404  
 1405  
 1406  
 1407  
 1408  
 1409  
 1410  
 1411  
 1412  
 1413  
 1414  
 1415  
 1416  
 1417  
 1418  
 1419  
 1420  
 1421  
 1422  
 1423  
 1424  
 1425  
 1426  
 1427  
 1428  
 1429  
 1430  
 1431  
 1432  
 1433  
 1434  
 1435  
 1436  
 1437  
 1438  
 1439  
 1440  
 1441  
 1442  
 1443  
 1444  
 1445  
 1446  
 1447  
 1448  
 1449  
 1450  
 1451  
 1452  
 1453  
 1454  
 1455  
 1456  
 1457  
 1458  
 1459  
 1460  
 1461  
 1462  
 1463  
 1464  
 1465  
 1466  
 1467  
 1468  
 1469  
 1470  
 1471  
 1472  
 1473  
 1474  
 1475  
 1476  
 1477  
 1478  
 1479  
 1480  
 1481  
 1482  
 1483  
 1484  
 1485  
 1486  
 1487  
 1488  
 1489  
 1490  
 1491  
 1492  
 1493  
 1494  
 1495  
 1496  
 1497  
 1498  
 1499  
 1500  
 1501  
 1502  
 1503  
 1504  
 1505  
 1506  
 1507  
 1508  
 1509  
 1510  
 1511  
 15

temperature and thereto 8.5 ml of triethylamine was added dropwise, whereupon the solution immediately turned into a violet solution. This solution was stirred at room temperature for 3 hours, then filtered and after adding thereto 20 ml of acetic acid and further adding 250 ml of ethyl acetate, stirred under ice cooling, as a result, crystals precipitated. The crystals were filtered and then washed with methanol and subsequently with acetone to obtain 4.30 g of crude crystals of Compound II-1. The crude crystals were dissolved in 80 ml of methanol and 3 ml of triethylamine and after adding thereto 5 ml of acetic acid, heated and then concentrated by distilling off the solvent. As a result, crystals precipitated. Thereafter, this solution was cooled with ice and the crystals were filtered, washed and dried to obtain 3.85 g of Compound II-1 (yield: 68%).

$\lambda_{\text{max}}$  (MeOH)=548.7 nm

#### Synthesis Example 2

##### (Synthesis of Compound III-1)

To 50 ml of methanol, 4.65 g of 4-{2-(2-ethoxy-1-butenyl)-5-fluoro-3-benzothiazolio}butanesulfonate and 4.00 g of 5-chloro-3-methanesulfonylcarbamoylmethyl-2-methylenothiazolium bromide were added. The resulting solution was stirred at room temperature and thereto 8.5 ml of triethylamine was added dropwise, whereupon the solution immediately turned into a violet solution. This solution was stirred at room temperature for 3 hours, then filtered and after adding thereto 17 ml of acetic acid, stirred under ice cooling, as a result, crystals precipitated. The crystals were filtered and then washed with methanol and subsequently with acetone to obtain 4.50 g of crude crystals of Compound III-1. The crude crystals were dissolved in 80 ml of methanol and 3 ml of triethylamine and after adding thereto 5 ml of acetic acid, heated and then concentrated by distilling off the solvent. As a result, crystals precipitated. Thereafter, this solution was cooled with ice and the crystals were filtered, washed and dried to obtain 3.99 g of Compound III-1 (yield: 60%).

$\lambda_{\text{max}}$  (MeOH)=551.4 nm

The compound represented by formula (I), (II) or (III) of the present invention may be incorporated into the silver halide emulsion of the present invention by directly dissolving the compound in the emulsion or may be added to the emulsion after dissolving the compound in a solvent such as water, methanol, ethanol, propanol, acetone, methyl cellosolve, 2,2,3,3-tetrafluoropropanol, 2,2,2-45 trifluoroethanol, 3-methoxy-1-propanol, 3-methoxy-1-butanol, 1-methoxy-2-propanol or N,N-dimethylformamide, or a mixed solvent thereof.

Other than these, the compound may be incorporated by the method of dissolving a dye in a volatile organic solvent, dispersing the solution in water or hydrophilic colloid, and adding the dispersion into an emulsion described in U.S. Pat. No. 3,469,987, the method of dispersing a water-insoluble dye in a water-soluble solvent without dissolving it, and adding the dispersion to an emulsion described in JP-B-46-24185 (the term "JP-B" as used herein means an "examined Japanese patent publication"), the method of dissolving a dye in an acid and adding the resulting solution to an emulsion, or forming an aqueous solution while allowing an acid or base to be present together and then adding the aqueous solution to an emulsion described in JP-B-44-23389, JP-B-44-27555 and JP-B-57-22091, the method of forming an aqueous solution or colloid dispersion while allowing a surfactant to be present together and adding it to an emulsion described in U.S. Pat. Nos. 3,822,135 and 4,006,026, the method of dispersing a dye directly in a hydrophilic colloid and adding the resulting dispersion to an

emulsion described in JP-A-53-102733 (the term "JP-A" as used herein means an "unexamined published Japanese patent application") and JP-A-58-105141, or the method of dissolving a dye using a compound capable of red shifting, and adding the resulting solution to an emulsion described in JP-A-51-74624. For the dissolution, an ultrasonic wave may also be used.

The compound represented by formula (I), (II) or (III) of the present invention may be added to the silver halide emulsion of the present invention in any step during the preparation of the emulsion, which is heretofore recognized as useful. The addition may be performed at any time or step as long as it is before the coating of the emulsion, for example, during the formation of silver halide grains and/or before the desalting, during the desalting and/or after the desalting but before the initiation of chemical ripening as disclosed in U.S. Pat. Nos. 2,735,766, 3,628,960, 4,183,756 and 4,225,666, JP-A-58-184142 and JP-A-60-196749, immediately before or during the chemical ripening, or after the chemical ripening but before the coating as disclosed in JP-A-58-113920. Also, as disclosed in U.S. Pat. 4,225,666 and JP-A-58-7629, the same compound solely or in combination with a compound having a different structure may be added in parts, for example, during the grain formation and during or after the completion of chemical ripening, or before- or during the chemical ripening and after the completion of chemical ripening. When added in parts, the kind of the compound or the combination of compounds may be varied.

The added amount of the compound represented by formula (I), (II) or (III) of the present invention varies depending on the shape and size of silver halide grain, however, it is usually from  $1 \times 10^{-6}$  to  $1 \times 10^{-2}$  mol, preferably from  $2 \times 10^{-6}$  to  $8 \times 10^{-3}$  mol, more preferably from  $6 \times 10^{-6}$  to  $6 \times 10^{-3}$ , per mol of silver halide. The compound of the present invention may be used alone but is preferably used in combination with other spectral sensitizing dye.

The silver halide photographic light-sensitive material of the present invention is described in detail below.

The silver halide which can be used in the silver halide photographic light-sensitive material of the present invention may be any of silver bromide, silver iodobromide, silver iodochlorobromide, silver chlorobromide and silver chloride. Among these, preferred are silver bromide, silver iodobromide, silver chlorobromide iodochlorobromide and silver halide having high silver chloride content described in JP-A-2-42, more preferred are silver bromide and silver iodobromide.

The silver halide grain contained in the photographic emulsion may be a grain having a regular crystal form such as cubic, octahedral or tetradecahedral form, a grain having an irregular crystal form such as spherical or tabular form, or a mixture thereof. In the present invention, the emulsion suitably contains grains having the above-described regular crystal form in a proportion of 50% or more, preferably 70% or more, more preferably 90% or more.

The emulsion preferably comprises tabular grains having an aspect ratio of 3 or more, more preferably from 8 to 100.

The emulsion for use in the present invention can be prepared by the method described, for example, in P. Glafkides, *Chimie et Physique Photographique*, Paul Montel (1967), G. F. Duffin, *Photographic Emulsion Chemistry*, The Focal Press (1966), and V. L. Zelikman et al., *Making and Coating Photographic Emulsion*, The Focal Press (1964). More specifically, any of an acidic process, a neutral process and an ammonia process may be used, and the reaction form between a soluble silver salt and a soluble

halogen salt may be any of a single jet method, a double jet method and a combination thereof. Also, the grain can be formed in an atmosphere of excess silver ion (so-called reverse mixing method). As one mode of the double jet method, a so-called controlled double jet method where the pAg of a liquid phase in which the silver halide is formed is kept constant, may also be used. According to this method, the silver halide emulsion obtained can have a regular crystal form and a nearly uniform grain size.

The silver halide emulsion for use in the present invention is usually subjected to chemical sensitization and spectral sensitization. For the chemical sensitization, chemical sensitization using a chalcogen sensitizer (to speak specifically, sulfur sensitization represented by the addition of a labile sulfur compound, selenium sensitization by a selenium compound, and tellurium sensitization by a tellurium compound), noble metal sensitization represented by gold sensitization, and reduction sensitization may be used individually or in combination. Preferred examples of the compound for use in the chemical sensitization include those described in JP-A-62-215272, from page 18, right lower column to page 22, right upper column.

The silver halide emulsion for use in the present invention may contain various compounds or precursors thereof, for the purpose of preventing the fogging during the production, storage or photographic processing of a light-sensitive material or stabilizing the photographic capabilities. Specific preferred examples of such compounds include those described in JP-A-62-215272, pp. 39-72. Also, 5-arylamino-1,2,3,4-thatriazole compounds (the aryl residue has at least one -electron withdrawing group) described in EP-A-447647 may be preferably used.

With respect to various techniques and inorganic/organic materials which can be used in the silver halide photographic light-sensitive material of the present invention, those described in *Research Disclosure*, Nos. 308119 (1989) and 37038 (1995) may be generally used.

In addition, to speak more specifically, the technique and inorganic/organic material which can be used in color photographic light-sensitive materials to which the silver halide photographic emulsion of the present invention can be applied, are described in the following portions of EP-A-436938 and cited patents therein.

-continued

| Items                                   | Pertinent Portions                                                               |
|-----------------------------------------|----------------------------------------------------------------------------------|
| 5 10) Formalin scavenger                | page 149, lines 15 to 17                                                         |
| 11) Other additives                     | page 153, lines 38 to 47; EP-A-421453, from page 75, line 21 to page 84, line 56 |
| 12) Dispersion method                   | page 150, lines 4 to 24                                                          |
| 13) Support                             | page 150, lines 32 to 34                                                         |
| 14) Film thickness, physical properties | page 150, lines 35 to 49                                                         |
| 15) Color development                   | from page 150, line 50 to page 151, line 47                                      |
| 16) Desilvering                         | from page 151, line 48 to page 152, line 53                                      |
| 17) Automatic developing machine        | from page 152, line 54 to page 153, line 2                                       |
| 18) Water washing/stabilization         | page 153, lines 3 to 37                                                          |

The silver halide emulsion prepared according to the present invention can be used for both color photographic light-sensitive material and black-and-white light-sensitive material. Examples of the color photographic light-sensitive material include color paper, color photographing film and color reversal film, and examples of the black-and-white photographic light-sensitive material include X-ray film, general photographing film and printing light-sensitive material film. Among these, preferred is color reversal film.

The present invention can be preferably applied to silver halide color photographic light-sensitive materials having a transparent magnetic recording layer. The silver halide light-sensitive material having a magnetic recording may be prepared in such a manner that a previously heat-treated polyester thin layer support described in detail in JP-A-6-35118, JP-A-6-17528 and *JIII Journal of Technical Disclosure* No. 94-6023 (for example, a polyethylene aromatic dicarboxylate-base polyester support), having a thickness of from 50 to 300  $\mu\text{m}$ , preferably from 50 to 200  $\mu\text{m}$ , more preferably from 80 to 115  $\mu\text{m}$ , is heat treated (annealed) at a temperature of from 40°C. to a glass transition temperature for 1 to 1,500 hours, the support is then subjected to a surface treatment such as ultraviolet irradiation described in JP-B-43-2603, JP-B-43-2604 and JP-B-45-3828, corona discharge described in JP-B-48-5043 and JP-A-51-131576, and glow discharge described in JP-B-35-7578 and JP-B-46-43480, undercoating described in U.S. Pat. 5,326,689 is applied thereon, a subbing layer described in U.S. Pat. No. 2,761,791 is provided, if desired, and ferromagnetic particles described in JP-A-59-23505, JP-A-4-195726 and JP-A-6-59357 are coated thereon.

The magnetic layer may be coated like stripes as described in JP-A-4-124642 and JP-A-4-124645.

55 The support may further be subjected to an antistatic treatment described in JP-A-4-62543, if desired, and finally, a silver halide photographic emulsion is coated thereon. For the silver halide grain used here, those described in JP-A-4-166932, JP-A-3-41436 and JP-A-3-41437 may be used.

60 This silver halide photographic light-sensitive material is preferably manufactured according to a manufacture control method described in JP-B-4-86817 and the manufacturing data are preferably recorded thereon by the method described in JP-B-6-87146. After or before the recording, the light-sensitive material is cut into a film smaller in the width than conventional 135 size films, and two perforations are punched in one side per one small-format picture accord-

| Items                        | Pertinent Portions                                                                                                                        |
|------------------------------|-------------------------------------------------------------------------------------------------------------------------------------------|
| 1) Layer Structure           | from page 146, line 34 to page 147, line 25                                                                                               |
| 2) Silver halide emulsion    | from page 147, line 26 to page 148, line 12                                                                                               |
| 3) Yellow coupler            | from page 137, line 35 to page 146, line 33, page 149, lines 21 to 23                                                                     |
| 4) Magenta coupler           | page 149, lines 24 to 28; EP-A-421453, from page 3, line 5 to page 25, line 55                                                            |
| 5) Cyan coupler              | from page 149, lines 29 to 33; EP-A-432804, from page 3, line 28 to page 40, line 2                                                       |
| 6) Polymer coupler           | page 149, lines 34 to 38, EP-A-435334, from page 113, line 39 to page 123, line 37                                                        |
| 7) Colored coupler           | from page 53, line 42 to page 137, line 34; page 149, lines 39 to 45                                                                      |
| 8) Other functional couplers | from page 7, line 1 to page 53, line 41; from page 149, line 46 to page 150, line 3; EP-A-435334, from page 3, line 1 to page 29, line 50 |
| 9) Antiseptic                | page 150, lines 25 to 28                                                                                                                  |

ing to the method described in JP-A-4-125560 so as to match the format picture smaller than conventional films.

The thus-prepared film is loaded in a cartridge package described in JP-A-4-157459, a cartridge described in JP-A-5-210202, FIG. 9, a film patrone described in U.S. Pat. No. 4,221,479 or a cartridge described in U.S. Pat. Nos. 4,834,306, 4,834,366, 5,226,613 and 4,846,418, and then used.

The film cartridge or film patrone used here is preferably of such a type that the tongue can be housed as described in U.S. Pat. Nos. 4,848,693 and 5,317,355 in view of the light-shielding property.

Also, a cartridge having a lock mechanism described in U.S. Pat. No. 5,296,886, a cartridge capable of indicating the use state described in U.S. Pat. No. 5,347,334 or a cartridge having a function of preventing double exposure is preferably used.

Furthermore, a cartridge where the film can be easily loaded by merely inserting the film into the cartridge described in JP-A-6-85128 may also be used.

The thus-produced film cartridge may be used for various photographic enjoyments by performing the photographing and development processing to satisfy the object using a camera, a developing machine or a laboratory machine.

The film cartridge (patrone) can fully exert its function when, for example, a camera in a simple loading system described in JP-A-6-8886 and JP-A-6-99908, a camera having an automatic winding-up system described in JP-A-6-57398 and JP-A-6-101135, a camera where the film can be taken out and exchanged on the way of photographing described in JP-A-6-205690, a camera where the photographing information such as panorama photographing, high-vision photographing or normal photographing (capable of magnetic recording such that the print aspect ratio can be selected) can be magnetic recorded on the film described in JP-A-5-293138 and JP-A-5-283382, a camera having a function of preventing double exposure described in JP-A-6-101194 or a camera having a function to indicate the use state of the film or the like described JP-A-5-150577, is used.

The thus-photographed film may be processed in an automatic developing machine described in JP-A-6-222514 and JP-A-6-212545 and before, during or after the processing, the use method of magnetic recording on a film described in JP-A-6-95265 and JP-A-4-123054 may be used. Also, the print aspect ratio selecting function described in JP-A-5-19364 may be used.

At the time of development processing of the film, in the case of cine-type development, the film is spliced according to the method described in JP-A-5-119461 before the processing.

During or after the development processing, the film may be subjected to an attaching/detaching operation described in JP-A-6-148805.

After such processing, the film information may be converted into a print through back printing or front printing on a color paper according to the method described in JP-A-2-184835, JP-A-4-186335 and JP-A-6-79968.

Furthermore, the film may be returned to the user together with the index print and the cartridge for return described in JP-A-5-11353 and JP-A-5-232594.

The present invention is described below in greater detail by referring to the Examples, but the present invention should not be construed as being limited thereto.

#### EXAMPLE 1

##### (Preparation of Sample 101)

A multi-layer color light-sensitive material comprising a 127  $\mu\text{m}$ -thick undercoated cellulose triacetate film support

having thereon layers each having the following composition was manufactured and designated as Sample 101. The numerals each indicates the added amount per  $\text{m}^2$ . The effect of each compound added is not limited to the use described below.

##### First Layer: Antihalation Layer

|    |                                          |         |
|----|------------------------------------------|---------|
| 10 | Black colloidal silver                   | 0.10 g  |
|    | Gelatin                                  | 2.00 g  |
|    | Ultraviolet Absorbent U-1                | 0.20 g  |
|    | Ultraviolet Absorbent U-3                | 0.040 g |
|    | Ultraviolet Absorbent U-4                | 0.15 g  |
| 15 | High Boiling Point Organic Solvent Oil-1 | 0.10 g  |
|    | Dye D-4                                  | 1.0 mg  |
|    | Dye D-8                                  | 2.5 mg  |
|    | Fine crystal solid dispersion of Dye E-1 | 0.10 g  |

##### Second Layer: Interlayer

|    |                                          |         |
|----|------------------------------------------|---------|
| 25 | Gelatin                                  | 0.40 g  |
|    | Compound Cpd-C                           | 0.5 mg  |
|    | Compound Cpd-J                           | 1.5 mg  |
|    | Compound Cpd-K                           | 4.0 mg  |
|    | High Boiling Point Organic Solvent Oil-3 | 0.010 g |
|    | High Boiling Point Organic Solvent Oil-4 | 0.020 g |
| 30 | High Boiling Point Organic Solvent Oil-5 | 2.0 mg  |
|    | High Boiling Point Organic Solvent Oil-7 | 2.0 mg  |
|    | High Boiling Point Organic Solvent Oil-8 | 5.0 mg  |
|    | Dye D-7                                  | 2.5 mg  |

##### Third Layer: Interlayer

|    |                                          |           |         |
|----|------------------------------------------|-----------|---------|
| 35 | Yellow colloidal silver                  | as silver | 0.010 g |
|    | Gelatin                                  | 0.40 g    |         |
|    | Compound Cpd-M                           | 0.015 g   |         |
|    | High Boiling Point organic Solvent Oil-3 | 0.020 g   |         |

##### Fourth Layer: First Red-sensitive Emulsion Layer

|    |                                          |           |         |
|----|------------------------------------------|-----------|---------|
| 45 | Emulsion A                               | as silver | 0.20 g  |
|    | Emulsion B                               | as silver | 0.20 g  |
|    | Emulsion C                               | as silver | 0.15 g  |
|    | Gelatin                                  |           | 0.70 g  |
|    | Coupler C-1                              |           | 0.10 g  |
| 50 | Coupler C-2                              |           | 0.050 g |
|    | Coupler C-3                              |           | 0.050 g |
|    | Coupler C-9                              |           | 0.010 g |
|    | Coupler C-11                             |           | 0.050 g |
|    | Compound Cpd-C                           |           | 5.0 mg  |
|    | Compound Cpd-I                           |           | 0.020 g |
| 55 | Compound Cpd-J                           |           | 5.0 mg  |
|    | High Boiling Point Organic Solvent Oil-2 |           | 0.10 g  |
|    | Additive P-1                             |           | 0.10 g  |

##### Fifth Layer: Second Red-sensitive Emulsion Layer

|    |             |           |         |
|----|-------------|-----------|---------|
| 60 | Emulsion C  | as silver | 0.25 g  |
|    | Emulsion D  | as silver | 0.25 g  |
|    | Gelatin     |           | 0.70 g  |
|    | Coupler C-1 |           | 0.15 g  |
|    | Coupler C-2 |           | 0.050 g |

-continued

|                                          |         |
|------------------------------------------|---------|
| Coupler C-3                              | 0.020 g |
| Coupler C-11                             | 0.070 g |
| High Boiling Point Organic Solvent Oil-2 | 0.10 g  |
| Additive P-1                             | 0.10 g  |

## Sixth Layer: Third Red-sensitive Emulsion Layer

|                                          |           |         |
|------------------------------------------|-----------|---------|
| Emulsion E                               | as silver | 0.20 g  |
| Emulsion F                               | as silver | 0.25 g  |
| Gelatin                                  |           | 1.20 g  |
| Coupler C-1                              |           | 0.10 g  |
| Coupler C-2                              |           | 0.050 g |
| Coupler C-3                              |           | 0.20 g  |
| Coupler C-11                             |           | 0.30 g  |
| High Boiling Point Organic Solvent Oil-2 |           | 0.10 g  |
| High Boiling Point Organic Solvent Oil-9 |           | 0.20 g  |
| Compound Cpd-K                           |           | 2.0 mg  |
| Compound Cpd-F                           |           | 0.050 g |
| Additive P-1                             |           | 0.10 g  |

## Seventh Layer: Interlayer

|                                          |         |
|------------------------------------------|---------|
| Gelatin                                  | 0.60 g  |
| Additive M-1                             | 0.30 g  |
| Compound Cpd-I                           | 2.6 mg  |
| Dye D-5                                  | 0.020 g |
| Dye D-6                                  | 0.010 g |
| Compound Cpd-M                           | 0.040 g |
| Compound Cpd-O                           | 3.0 mg  |
| Compound Cpd-P                           | 2.5 mg  |
| High Boiling Point Organic Solvent Oil-1 | 0.020 g |
| High Boiling Point Organic Solvent Oil-6 | 0.050 g |

## Eighth Layer: Interlayer

|                                          |           |         |
|------------------------------------------|-----------|---------|
| Yellow colloidal silver                  | as silver | 0.010 g |
| Gelatin                                  |           | 0.60 g  |
| Additive P-1                             |           | 0.05 g  |
| Compound Cpd-A                           |           | 0.10 g  |
| Compound Cpd-M                           |           | 0.10 g  |
| High Boiling Point Organic Solvent Oil-6 |           | 0.10 g  |

## Ninth Layer: First Green-sensitive Layer

|                                          |           |          |
|------------------------------------------|-----------|----------|
| Emulsion G                               | as silver | 0.25 g   |
| Emulsion H                               | as silver | 0.30 g   |
| Emulsion I                               | as silver | 0.25 g   |
| Gelatin                                  |           | 1.00 g   |
| Coupler C-7                              |           | 0.10 g   |
| Coupler C-8                              |           | 0.17 g   |
| Compound Cpd-B                           |           | 0.300 g  |
| Compound Cpd-D                           |           | 0.020 g  |
| Compound Cpd-E                           |           | 0.020 g  |
| Compound Cpd-G                           |           | 2.5 mg   |
| Compound Cpd-F                           |           | 0.040 mg |
| Compound Cpd-K                           |           | 2.0 mg   |
| Compound Cpd-L                           |           | 0.020 g  |
| High Boiling Point Organic Solvent Oil-1 |           | 0.05 g   |
| High Boiling Point Organic Solvent Oil-2 |           | 0.10 g   |

## Tenth Layer: Second Green-sensitive Layer

|    |                                          |           |         |
|----|------------------------------------------|-----------|---------|
| 5  | Emulsion I                               | as silver | 0.20 g  |
|    | Emulsion J                               | as silver | 0.20 g  |
|    | Gelatin                                  |           | 0.70 g  |
|    | Coupler C-4                              |           | 0.25 g  |
|    | Compound Cpd-B                           |           | 0.030 g |
|    | Compound Cpd-D                           |           | 0.020 g |
|    | Compound Cpd-F                           |           | 0.050 g |
| 10 | Compound Cpd-G                           |           | 2.0 mg  |
|    | High Boiling Point Organic Solvent Oil-2 |           | 0.10 g  |

## Eleventh Layer: Third Green-sensitive Layer

|    |                                          |           |         |
|----|------------------------------------------|-----------|---------|
| 15 | Emulsion K                               | as silver | 0.55 g  |
|    | Gelatin                                  |           | 0.80 g  |
|    | Coupler C-4                              |           | 0.35 g  |
|    | Compound Cpd-B                           |           | 0.080 g |
|    | Compound Cpd-D                           |           | 0.020 g |
|    | Compound Cpd-F                           |           | 0.040 g |
|    | Compound Cpd-K                           |           | 5.0 mg  |
|    | High Boiling Point Organic Solvent Oil-2 |           | 0.15 g  |

## Twelfth Layer: Interlayer

|    |                                          |         |
|----|------------------------------------------|---------|
| 30 | Gelatin                                  | 0.30 g  |
|    | Compound Cpd-M                           | 0.05 g  |
|    | High Boiling Point Organic Solvent Oil-3 | 0.025 g |
|    | High Boiling Point Organic Solvent Oil-6 | 0.025 g |

## Thirteenth Layer: Yellow Filter Layer

|    |                                          |           |         |
|----|------------------------------------------|-----------|---------|
| 40 | Yellow colloidal silver                  | as silver | 5.0 mg  |
|    | Gelatin                                  |           | 1.00 g  |
|    | Compound Cpd-C                           |           | 0.010 g |
|    | Compound Cpd-M                           |           | 0.030 g |
|    | Compound Cpd-L                           |           | 0.010 g |
|    | High Boiling Point Organic Solvent Oil-1 |           | 0.020 g |
| 45 | Fine crystal solid dispersion of Dye E-2 |           | 0.030 g |
|    | Fine crystal solid dispersion of Dye E-3 |           | 0.020 g |

## Fourteenth Layer: Interlayer

|    |         |        |
|----|---------|--------|
| 50 | Gelatin | 0.40 g |
|    |         |        |

## Fifteenth Layer: First Blue-sensitive Layer

|    |                |           |         |
|----|----------------|-----------|---------|
| 55 | Emulsion L     | as silver | 0.20 g  |
|    | Emulsion M     | as silver | 0.20 g  |
|    | Gelatin        |           | 0.80 g  |
|    | Coupler C-5    |           | 0.20 g  |
|    | Coupler C-6    |           | 0.10 g  |
|    | Coupler C-10   |           | 0.10 g  |
|    | Compound Cpd-I |           | 0.010 g |
| 60 | Compound Cpd-M |           | 0.010 g |
|    |                |           |         |

## Sixteenth Layer: Second Blue-sensitive Layer

|                                          |           |         |  |
|------------------------------------------|-----------|---------|--|
| Emulsion N                               | as silver | 0.20 g  |  |
| Emulsion O                               | as silver | 0.20 g  |  |
| Gelatin                                  |           | 0.90 g  |  |
| Coupler C-5                              |           | 0.10 g  |  |
| Coupler C-6                              |           | 0.10 g  |  |
| Coupler C-10                             |           | 0.10 g  |  |
| Compound Cpd-N                           |           | 2.0 mg  |  |
| Compound Cpd-K                           |           | 2.0 mg  |  |
| High Boiling Point Organic Solvent Oil-2 |           | 0.050 g |  |

## Seventeenth Layer: Third Blue-sensitive Layer

|                                          |           |        |  |
|------------------------------------------|-----------|--------|--|
| Emulsion O                               | as silver | 0.20 g |  |
| Emulsion P                               | as silver | 0.25 g |  |
| Gelatin                                  |           | 1.20 g |  |
| Coupler C-5                              |           | 0.10 g |  |
| Coupler C-6                              |           | 0.10 g |  |
| Coupler C-10                             |           | 0.80 g |  |
| High Boiling Point Organic Solvent Oil-2 |           | 0.10 g |  |
| Compound Cpd-N                           |           | 5.0 mg |  |
| Compound Cpd-Q                           |           | 0.20 g |  |

## Eighteenth Layer: First Protective Layer

|                           |         |  |
|---------------------------|---------|--|
| Gelatin                   | 0.70 g  |  |
| Ultraviolet Absorbent U-1 | 0.20 g  |  |
| Ultraviolet Absorbent U-2 | 0.050 g |  |
| Ultraviolet Absorbent U-5 | 0.30 g  |  |
| Compound Cpd-O            | 5.0 mg  |  |
| Compound Cpd-A            | 0.030 g |  |
| Compound Cpd-H            | 0.20 g  |  |
| Dye D-1                   | 0.10 g  |  |
| Dye D-2                   | 0.050 g |  |
| Dye D-3                   | 0.07 g  |  |

-continued

|   |                                          |        |
|---|------------------------------------------|--------|
| 5 | High Boiling Point Organic Solvent Oil-3 | 0.10 g |
|---|------------------------------------------|--------|

## Nineteenth Layer: Second Protective Layer

|    |                                                                                                        |           |         |
|----|--------------------------------------------------------------------------------------------------------|-----------|---------|
| 10 | Colloidal silver                                                                                       | as silver | 0.10 mg |
|    | Fine grain silver iodobromide emulsion (average grain size: 0.06 $\mu\text{m}$ , AgI content: 1 mol %) | as silver | 0.10 g  |
|    | Gelatin                                                                                                |           | 0.50 g  |

## Twelfth Layer: Third Protective Layer

|    |                                                                                                       |         |
|----|-------------------------------------------------------------------------------------------------------|---------|
| 20 | Gelatin                                                                                               | 0.80 g  |
|    | Polymethyl methacrylate (average particle size 1.5 $\mu\text{m}$ )                                    | 0.10 g  |
|    | 6:4 Copolymer of methyl methacrylate and methacrylic acid (average particle size: 1.5 $\mu\text{m}$ ) | 0.10 g  |
|    | Silicone Oil SO-1                                                                                     | 0.030 g |
| 25 | Surfactant W-1                                                                                        | 3.0 mg  |
|    | Surfactant W-2                                                                                        | 0.030 g |
|    | Surfactant W-7                                                                                        | 2.5 mg  |

30 In addition to the above-described compositions, a gelatin hardener H-1 and surfactants W-3, W-4, W-5 and W-6 for coating and emulsification were added to each layer.

Furthermore, phenol, 1,2-benzoisothiazolin-3-one, 2-phenoxyethanol, phenethyl alcohol and p-hydroxybenzoic acid butyl ester as antiseptic or antifungal were added to each layer.

35 The light-sensitive emulsions used in Sample 101 are shown in Tables 1 and 2.

TABLE 1

## Silver Iodobromide Emulsion Used in Sample 101

| Emulsion | Characteristic Features                                                                 | Equivalent-Sphere Average Grain Size ( $\mu\text{m}$ ) | Variation Coefficient (%) | AgI Content (%) |
|----------|-----------------------------------------------------------------------------------------|--------------------------------------------------------|---------------------------|-----------------|
| A        | monodisperse tetradechedral grain                                                       | 0.13                                                   | 10                        | 4.0             |
| B        | monodisperse (100) tabular grain, average aspect ratio: 10                              | 0.25                                                   | 12                        | 3.8             |
| C        | monodisperse (111) tabular grain (internal latent image type), average aspect ratio: 12 | 0.30                                                   | 13                        | 3.8             |
| D        | monodisperse (111) tabular grain, average aspect ratio: 10                              | 0.35                                                   | 17                        | 4.8             |
| E        | monodisperse (111) tabular grain, average aspect ratio: 3                               | 0.40                                                   | 15                        | 2.0             |
| F        | monodisperse (111) tabular grain, average aspect ratio: 20                              | 0.50                                                   | 12                        | 1.8             |
| G        | monodisperse cubic grain                                                                | 0.15                                                   | 9                         | 3.5             |
| H        | monodisperse (100) tabular grain, average aspect ratio: 10                              | 0.24                                                   | 12                        | 3.5             |
| I        | monodisperse (111) tabular grain, average aspect ratio: 10                              | 0.31                                                   | 16                        | 3.5             |
| J        | monodisperse (111) tabular grain, average aspect ratio: 15                              | 0.45                                                   | 16                        | 3.0             |
| K        | monodisperse (111) tabular grain, average aspect ratio: 20                              | 0.60                                                   | 15                        | 3.3             |
| L        | monodisperse tetradechedral grain                                                       | 0.33                                                   | 10                        | 4.5             |
| M        | monodisperse (100) tabular grain, average aspect ratio: 11                              | 0.33                                                   | 8                         | 4.5             |
| N        | monodisperse (111) tabular grain, average aspect ratio: 15                              | 0.43                                                   | 10                        | 2.5             |

TABLE 1-continued

| Silver Iodobromide Emulsion Used in Sample 101 |                                                            |                                                        |                           |                 |
|------------------------------------------------|------------------------------------------------------------|--------------------------------------------------------|---------------------------|-----------------|
| Emulsion                                       | Characteristic Features                                    | Equivalent-Sphere Average Grain Size ( $\mu\text{m}$ ) | Variation Coefficient (%) | AgI Content (%) |
| O                                              | monodisperse (111) tabular grain, average aspect ratio: 20 | 0.75                                                   | 9                         | 2.0             |
| P                                              | monodisperse (111) tabular grain, average aspect ratio: 25 | 0.90                                                   | 8                         | 1.8             |

TABLE 2

| Emulsion | Sensitizing Dye Added | Added Amount per 1 mol of Silver Halide (g) |
|----------|-----------------------|---------------------------------------------|
| A        | S-1                   | 0.26                                        |
|          | S-7                   | 0.025                                       |
| B        | S-1                   | 0.265                                       |
|          | S-7                   | 0.025                                       |
| C        | S-1                   | 0.23                                        |
|          | S-7                   | 0.025                                       |
| D        | S-1                   | 0.205                                       |
|          | S-7                   | 0.10                                        |
| E        | S-1                   | 0.19                                        |
|          | S-7                   | 0.10                                        |
| F        | S-1                   | 0.22                                        |
|          | S-7                   | 0.025                                       |
| G        | S-5                   | 0.35                                        |
|          | S-8                   | 0.12                                        |
| H        | S-5                   | 0.23                                        |
|          | S-8                   | 0.12                                        |
| I        | S-2                   | 0.1                                         |
|          | S-5                   | 0.29                                        |
| J        | S-5                   | 0.18                                        |
|          | S-8                   | 0.18                                        |
| K        | S-2                   | 0.050                                       |
|          | S-5                   | 0.34                                        |
| L        | S-3                   | 0.25                                        |
|          | S-4                   | 0.20                                        |
| M        | S-3                   | 0.10                                        |
|          | S-4                   | 0.15                                        |
| N        | S-6                   | 0.25                                        |
|          | S-4                   | 0.25                                        |
| O        | S-6                   | 0.25                                        |
|          | S-3                   | 0.10                                        |
| P        | S-4                   | 0.20                                        |
|          | S-6                   | 0.25                                        |
| P        | S-3                   | 0.050                                       |
|          | S-4                   | 0.25                                        |
|          | S-6                   | 0.25                                        |

TABLE 2-continued

15 Note 1) The emulsions all were chemically sensitized using gold, sulfur and selenium.

20 Note 2) In all of the emulsions, sensitizing dyes were added before the chemical sensitization.

25 Note 3) In the emulsions, Compounds F-1, F-2, F-3, F-4, F-5, F-6, F-7, F-8, F-9 or F-10 was appropriately added.

(Preparation of Dispersion of Organic Solid Disperse Dye)

30 Dye E-1 was dispersed in the following manner. To 1,430 g of a dye wet cake containing 30% of water, water and W-4 were added each in an amount of 70 g. This mixture was stirred to form a slurry having a dye concentration of 6%. Thereafter, to Ultravisco Mill (UVM-2) manufactured by

35 Imex, 1,700 ml of zirconia beads having an average particle size of 0.5 mm were filled and the slurry was passed therethrough and pulverized at a peripheral speed of about 10 m/sec with a discharge amount of 0.5 l/min over 8 hours. Thereafter, beads were removed by filtration and the dye

40 particles obtained were heated for the stabilization at 90° C. for 10 hours and then diluted by adding water and gelatin to a dye concentration of 3%. The obtained dye fine particles had an average particle size of 0.60  $\mu\text{m}$  and a particle size distribution width (standard deviation of particle size  $\times 10$ /average particle size) of 18%.

Solid dye dispersions of Dyes E-2 and E-3 were obtained in the same manner. These had an average particle size of 0.54  $\mu\text{m}$  and 0.56  $\mu\text{m}$ , respectively.

(Preparation of Samples 100 and 102 to 108)

45 Samples 102 to 108 were prepared by replacing only Sensitizing Dye S-1 in Emulsions A to F of Sample 101 to an amount (molar times) shown in Table 3. Also, Dye Blank Sample 100 was prepared by omitting the dyes.

C-1



C-2



**29****30**

-continued

C-3



C-4

Numerals are wt%.  
Average molecular weight:  
about 25,000

C-5



C-6



C-7



C-8



C-9



C-10



-continued

C-11

Dibutyl phthalate

Oil-1



Tricresyl phosphate

Oil-2



Oil-3

Tricyclohexyl phosphate

Oil-4

Dicyclohexyl phthalate

Oil-5

Oil-6



Oil-7



Oil-8



Oil-9



Cpd-A



Cpd-B



Cpd-C



Cpd-D



-continued

Cpd-E



Cpd-F



Cpd-G

Cpd-H

Cpd-I



Cpd-K

Cpd-L

Cpd-M



Cpd-N

Cpd-O



Cpd-P

Cpd-Q



U-1



-continued

U-2



U-3

U-4



U-5

S-1



S-2

S-3



S-4

S-5



S-6

S-7



S-8

S-9



D-1



**37****38**

-continued

D-2



D-3

D-4



D-5



D-6



D-7



D-8



E-1







-continued

F-6



F-8



F-7

F-9

F-10

## (Evaluation of Residual Color and Photographic Property)

The thus-obtained samples each was exposed to white light through a gray wedge for  $\frac{1}{100}$  second at 20 CMS, processed according to the processing steps shown below, and then subjected to sensitometry. The residual color was evaluated by subtracting the density of magenta stain of Dye Blank Sample 100 from the magenta density in stain of each processed sample. The stain density was measured by a density measuring device, Status A, manufactured by X-RITE. (Processing)

25

-continued

|    |                              | Tank Solution | Replenisher |
|----|------------------------------|---------------|-------------|
| 30 | hydroxymethyl-3-pyrazolidone | 2.5 g         | 1.4 g       |
|    | Potassium bromide            | 1.2 g         | 1.2 g       |
|    | Potassium thiocyanate        | 2.0 mg        | —           |
|    | Potassium iodide             | 13 g          | 15 g        |
| 35 | Diethylene glycol            | 1000 ml       | 1000 ml     |
|    | Water to make                | 9.60          | 9.60        |
|    | pH                           |               |             |

The pH was adjusted with sulfuric acid or potassium hydroxide.

## (Reversal Solution)

|    |                                                             | Tank Solution | Replenisher           |
|----|-------------------------------------------------------------|---------------|-----------------------|
| 45 | Nitrilo-N,N,N-trimethylene phosphonic acid pentasodium salt | 3.0 g         | same as tank solution |
|    | Stannous chloride dihydrate                                 | 1.0 g         |                       |
|    | p-Aminophenol                                               | 0.1 g         |                       |
|    | Sodium hydroxide                                            | 8 g           |                       |
| 50 | Glacial acetic acid                                         | 15 ml         |                       |
|    | Water to make                                               | 1000 ml       |                       |
|    | pH                                                          | 6.00          |                       |

The pH was adjusted with acetic acid or sodium hydroxide.

## (Color Developer)

|    |                                                             | Tank Solution | Replenisher |
|----|-------------------------------------------------------------|---------------|-------------|
| 60 | Nitrilo-N,N,N-trimethylene phosphonic acid pentasodium salt | 2.0 g         | 2.0 g       |
|    | Diethylenetriaminepentaacetic acid pentasodium salt         | 7.0 g         | 7.0 g       |
|    | Sodium sulfite                                              | 36 g          | 36 g        |
|    | Potassium hydroquinone monosulfonate                        | 1.0 g         | —           |
| 65 | Phosphoric acid trisodium dodecahydrate                     | 90 mg         | —           |
|    | Potassium bromide                                           |               |             |
|    | Potassium iodide                                            |               |             |

-continued

|                                                                       | Tank<br>Solution | Re-<br>plenisher |   |
|-----------------------------------------------------------------------|------------------|------------------|---|
| Sodium hydroxide                                                      | 3.0 g            | 3.0 g            |   |
| Citrazinic acid                                                       | 1.5 g            | 1.5 g            |   |
| N-Ethyl-N-( $\beta$ -methanesulfonamidoethyl)-3-methyl-4-aminoaniline | 11 g             | 11 g             |   |
| 3/2 sulfuric acid monohydrate                                         |                  |                  | 5 |
| 3,6-Dithiaoctane-1,8-diol                                             | 1.0 g            | 1.0 g            |   |
| Water to make                                                         | 1000 ml          | 1000 ml          |   |
| pH                                                                    | 11.80            | 12.00            |   |

The pH was adjusted with sulfuric acid or potassium hydroxide.

(Stabilizing Solution)

|                                                                                    | Tank<br>Solution | Re-<br>plenisher |
|------------------------------------------------------------------------------------|------------------|------------------|
| 1,2-Benzothiazolin-3-one                                                           | 0.02 g           | 0.03 g           |
| Polyoxyethylene-p-<br>monononylphenyl ether (average<br>polymerization degree: 10) | 0.3 g            | 0.3 g            |
| Polymaleic acid (average<br>molecular weight: 2,000)                               | 0.1 g            | 0.15 g           |
| Water to make                                                                      | 1000 ml          | 1000 ml          |
| pH                                                                                 | 7.0              | 7.0              |

## (Pre-Bleaching Solution)

|                                                            | Tank<br>Solution | Re-<br>plenisher |    |
|------------------------------------------------------------|------------------|------------------|----|
| Ethylenediaminetetraacetic acid<br>disodium salt dihydrate | 8.0 g            | 8.0 g            |    |
| Sodium sulfite                                             | 6.0 g            | 8.0 g            | 20 |
| 1-Thioglycerol                                             | 0.4 g            | 0.4 g            |    |
| Formaldehyde sodium bisulfite<br>adduct                    | 30 g             | 35 g             |    |
| Water to make                                              | 1000 mg          | 1000 ml          |    |
| pH                                                         | 6.30             | 6.10             |    |

The pH was adjusted with acetic acid or sodium hydroxide.

## (Bleaching Solution)

|                                                               | Tank<br>Solution | Re-<br>plenisher |    |
|---------------------------------------------------------------|------------------|------------------|----|
| Ethylenediaminetetraacetic acid<br>disodium salt dihydrate    | 2.0 g            | 4.0 g            | 40 |
| Ethylenediaminetetraacetic acid<br>Fe(III) ammonium dihydrate | 120 g            | 240 g            |    |
| Potassium bromide                                             | 100 g            | 200 g            |    |
| Ammonium nitrate                                              | 10 g             | 20 g             |    |
| Water to make                                                 | 1000 ml          | 1000 ml          |    |
| pH                                                            | 5.70             | 5.50             |    |

The pH was adjusted with nitric acid or sodium hydroxide.

## (Fixing Solution)

|                      | Tank<br>Solution | Replenisher                 |    |
|----------------------|------------------|-----------------------------|----|
| Ammonium thiosulfate | 80 g             | Same as<br>tank<br>solution | 55 |
| Sodium sulfite       | 5.0 g            | Same as<br>tank<br>solution |    |
| Sodium bisulfite     | 5.0 g            | Same as<br>tank<br>solution | 60 |
| Water to make        | 1000 ml          | 1000 ml                     |    |
| pH                   | 6.60             |                             |    |

The pH was adjusted with acetic acid or aqueous ammonia.

The evaluation results of the sensitometry and residual color are shown in Table 3 below. The relative sensitivity RL was compared based on the relative exposure amount necessary for giving a density 1.0 larger than the minimum density.

TABLE 3

| Sam-<br>ple<br>No. | Dye   | $\pi_v$ | $\pi_w$ | Dye<br>amount<br>(molar<br>times) | RL,<br>relative<br>sensitivity | Magenta<br>Residual<br>Color<br>Density | Remarks         |
|--------------------|-------|---------|---------|-----------------------------------|--------------------------------|-----------------------------------------|-----------------|
| 100                | none  |         |         |                                   |                                | 0 (control)                             | Blank           |
| 101                | S-1   | 0.71    | 0.71    | $\times 1$                        | 100                            | 0.062                                   | Com-<br>parison |
| 102                | S-9   | 0.71    | 0.71    | $\times 1.1$                      | 98                             | 0.058                                   | Com-<br>parison |
| 103                | I-11  | 0.71    | 0.14    | $\times 1.2$                      | 105                            | 0.040                                   | Invention       |
| 104                | I-16  | 0.14    | 0.14    | $\times 1.3$                      | 100                            | 0.031                                   | Invention       |
| 105                | II-1  | 0.14    | 0.71    | $\times 1.2$                      | 113                            | 0.028                                   | Invention       |
| 106                | II-2  | 0.71    | 0.00    | $\times 1.2$                      | 108                            | 0.020                                   | Invention       |
| 107                | III-1 | 0.14    | 0.71    | $\times 1$                        | 101                            | 0.018                                   | Invention       |
| 108                | III-1 | 0.14    | 0.71    | $\times 1.2$                      | 115                            | 0.025                                   | Invention       |

As is apparent from the results in Table 3, by using compound of the present invention, a light-sensitive material reduced in the residual color and having high sensitivity can be obtained. Thus, it is clearly verified that by virtue of the construction of the present invention, both high sensitivity and reduced residual color can be first attained.

By the construction of the present invention, a silver halide photographic light-sensitive material having high sensitivity and reduced in the residual color can be obtained.

While the invention has been described in detail and with reference to specific embodiments thereof, it will be apparent to one skilled in the art that various changes and modifications can be made therein without departing from the spirit and scope thereof.

What is claimed is:

1. A silver halide photographic light-sensitive material comprising a support having provided thereon at least one emulsion layer containing silver halide grains, which comprises at least one compound represented by the following formula (I):



wherein  $Z_1$  and  $Z_2$  each represents an oxygen atom, a sulfur atom, a selenium atom, a tellurium atom or a  $>NR$  group,  $R$  represents an alkyl group, an aryl group or a heterocyclic group,  $L_1$ ,  $L_2$  and  $L_3$  each represents a methine group,  $n_1$  represents 0, 1, 2 or 3,  $V_1$ ,  $V_2$ ,  $V_3$ ,  $V_4$ ,  $W_1$ ,  $W_2$ ,  $W_3$  and  $W_4$  each represents a hydrogen atom or a substituent, provided that two substituents may be combined with each other to form a condensed ring on the condition that assuming the sum total of  $\pi$  values of the substituents  $V_1$  to  $V_4$  is  $\pi_v$  and the sum total of  $\pi$  values of the substituents  $W_1$  to  $W_4$  is  $\pi_w$ , either one of  $\pi_v$  and  $\pi_w$  is 0.70 or less and the other is 0.70 or more,  $M$  represents a charge-balancing counter ion,  $m$  represents a number necessary for neutralizing the electric charge of the molecule,  $R_1$  represents an alkyl group, an aryl group or a heterocyclic group, and  $R_2$  represents a substituent represented by the following formula:



wherein  $L_e$  represents a methylene group, and  $k_e$  represents an integer of 1 or more.

2. The silver halide photographic light-sensitive material as claimed in claim 1, wherein  $\pi_v$  is 0.70 or less and  $\pi_w$  is 0.70 or more.

3. The silver halide photographic light-sensitive material as claimed in claim 2, wherein  $\pi_v$  is from 0.00 to 0.70 and  $\pi_w$  is 0.70 to 1.40.

4. The silver halide photographic light-sensitive material as claimed in claim 1, wherein the compound represented by formula (I) is a compound represented by the following formula (II):



wherein  $Z_3$  and  $Z_4$  each represents oxygen atom or sulfur atom,  $A_1$  represents hydrogen atom or an alkyl group, either one of  $V_5$  and  $W_5$  is a substituent selected from the group consisting of chlorine atom, bromine atom, iodine atom, a trifluoromethyl group, an ethyl group, a benzoyl group and a 1-pyrrolyl group, and the other is a substituent selected from the group consisting of hydrogen atom, fluorine atom, a methyl group, a methylthio group, an ethoxy group, an ethoxycarbonyl group, a 2-pyridyl group and a 4-pyridyl group,  $M_1$  represents a charge-balancing counter ion,  $m_1$  represents a number necessary for neutralizing the electric charge of the molecule,  $R_3$  represents an alkyl group having a sulfo group as a substituent,  $L_f$  represents a methylene group, and  $k_f$  represents an integer of from 1 to 3.

5. A silver halide photographic light-sensitive material comprising a support having provided thereon at least one emulsion layer containing silver halide grains, which comprises at least one compound represented by the following formula (I)



wherein  $Z_1$  and  $Z_2$  each represents oxygen atom, sulfur atom, selenium atom, tellurium atom or a  $>NR$  group,  $R$  represents an alkyl group, an aryl group or a heterocyclic group,  $L_1$ ,  $L_2$  and  $L_3$  each represents a methine group,  $n_1$  represents 0, 1, 2 or 3,  $V_1$ ,  $V_2$ ,  $V_3$ ,  $V_4$ ,  $W_1$ ,  $W_2$ ,  $W_3$  and  $W_4$  each represents a hydrogen atom or a substituent, provided that two substituents may be combined with each other to form a condensed ring on the condition that assuming the sum total of  $\pi$  values of the substituents  $V_1$  to  $V_4$  is  $\pi_v$ , and the sum total of  $\pi$  values of the substituents  $W_1$  to  $W_4$  is  $\pi_w$ ,  $\pi_v$  is from 0.00 to 0.70 and  $\pi_w$  is from 0.70 to 1.40,  $M$  represents a charge-balancing counter ion,  $m$  represents a number necessary for neutralizing the electric charge of the molecule,  $R_1$  represents an alkyl group, an aryl group or a heterocyclic group, and  $R_2$  represents a substituent represented by any one of the following formulae:



wherein  $R_a$ ,  $R_b$ ,  $R_c$  and  $R_d$  each represents an alkyl group, an aryl group, a heterocyclic group, an alkoxy group, an aryloxy group, a heterocyclyloxy group or an amino group,  $L_a$ ,  $L_b$ ,  $L_c$  and  $L_d$  each represents a methylene group, and  $k_a$ ,  $k_b$ ,  $k_c$  and  $k_d$  each represents an integer of 1.

6. The silver halide photographic light-sensitive material, as claimed in claim 5, wherein the compound represented by formula (I) is a compound represented by the following formula (III):



wherein  $Z_5$  and  $Z_6$  each represents oxygen atom or sulfur atom,  $A_2$  represents hydrogen atom or an alkyl group,  $V_6$  represents a substituent selected from the group consisting of hydrogen atom, fluorine atom, a methyl group, a methylthio group, an ethoxy group, an ethoxycarbonyl group, a 2-pyridyl group and a 4-pyridyl group,  $M_2$  represents a charge-balancing counter ion,  $m_2$  represents a number necessary for neutralizing the electric charge of the molecule,  $R_g$  represents an alkyl group having a sulfo group as a substituent, and  $k_g$  represents an integer of from 1 to 3.

substituent selected from the group consisting of chlorine atom, bromine atom, iodine atom, a trifluoromethyl group, an ethyl group, a benzoyl group and a 1-pyrrolyl group,  $M_2$  represents a charge-balancing counter ion,  $m_2$  represents a number necessary for neutralizing the electric charge of the molecule,  $R_4$  represents an alkyl group having a sulfo group as a substituent,  $R_g$  represents an alkyl group,  $L_g$  represents a methylene group, and  $k_g$  represents an integer of 1.

7. The silver halide photographic light-sensitive material as claimed in claim 1, 2, 3, 4, 5, or 6, wherein at least one compound represented by formula (I) (II) or (III) is contained and the emulsion layer containing said compound is formed of silver halide grains having an average aspect ratio of from 3 to 100.

\* \* \* \* \*